# EUROPEAN PATENT SPECIFICATION

(11) **EP 4 528 382 B1**
(45) Date of publication and mention of the grant of the patent: **29.10.2025**
(21) Application number: 24159593.3
(22) Date of filing: 26.02.2024
(51) Int. Cl.: G03G 5/06, G03G 5/14

(54) **ELECTROPHOTOGRAPHIC PHOTORECEPTOR, PROCESS CARTRIDGE, AND IMAGE FORMING APPARATUS**
ELEKTROPHOTOGRAPHISCHER PHOTOREZEPTOR, PROZESSKARTUSCHE UND BILDERZEUGUNGSVORRICHTUNG
PHOTORÉCEPTEUR ÉLECTROPHOTOGRAPHIQUE, CARTOUCHE DE TRAITEMENT ET APPAREIL DE FORMATION D'IMAGE

(30) Priority: 25.09.2023 JP 2023161679
(43) Date of publication of application: 26.03.2025
(73) Proprietor: FUJIFILM Business Innovation Corp., Minato-ku Tokyo (JP)
(72) Inventor: IWASAKI, Masahiro, Minamiashigara-shi, Kanagawa (JP); OYAMADA, Yuki, Ebina-shi, Kanagawa (JP)
(74) Representative: Becker Kurig & Partner Patentanwälte mbB

(56) References cited:
- WO-A1-2005/092901
- US-B2- 10 065 969

## Description

### BACKGROUND OF THE INVENTION

### (i) Field of the Invention

The present invention relates to an electrophotographic photoreceptor, a process cartridge, and an image forming apparatus.

### (ii) Description of Related Art

In an electrophotographic image forming apparatus, typically, a surface of an electrophotographic photoreceptor is charged to a predetermined polarity and a predetermined potential using a charging unit, the charges of the charged surface of the electrophotographic photoreceptor are selectively erased by performing image exposure to light to form an electrostatic latent image, a toner is made to adhere to the electrostatic latent image using a developing unit, and the latent image is developed as a toner image. Further, the toner image is transferred to a medium to be transferred by a transfer unit to discharge an image formed product. In recent years, electrophotographic photoreceptors have advantages that a high speed and a high print quality can be obtained, and thus have been widely used in the fields such as copying machines and laser beam printers.

Recently, an electrophotographic photoreceptor is formed such that an undercoat layer is formed on a conductive support layer such as an aluminum base material, and a single layer type photosensitive layer containing a charge generation agent and a charge transport agent in the same layer or a so-called function separation type photosensitive layer obtained by laminating a charge generation layer containing a charge generation agent and a charge transport layer containing a charge transport agent containing a charge transport agent are sequentially formed on the undercoat layer.

The undercoat layer is required to cover defects of the base material, suppress charge injection to the photosensitive layer in a case of application of a voltage to the electrophotographic photoreceptor, and control the resistance. Meanwhile, the undercoat layer is also required to suppress the charge generated by the photosensitive layer from staying inside the photoreceptor, that is, to have charge transport properties.

JP3991638B discloses an electrophotographic photoreceptor including a conductive support layer, a photosensitive layer containing a pigment, and an interlayer disposed between the conductive support layer and the photosensitive layer, in which the interlayer contains zinc oxide particles and a binder resin, a maximum value of a primary particle diameter of the zinc oxide particles contained in the interlayer is less than 300 nm, an average particle diameter thereof is in a range of 20 to 200 nm, and the interlayer has a layer thickness of 15 to 50 µm.

JP2003-091086A discloses an electrophotographic photoreceptor including a conductive support layer, a photosensitive layer containing a pigment, and an interlayer disposed between the conductive support layer and the photosensitive layer, in which the interlayer contains metal oxide particles subjected to a coating treatment with a coupling agent and a binder resin, the interlayer has a layer thickness of greater than 20 µm and 50 µm or less, and the binder resin is a thermosetting resin.

JP2003-330209A discloses an electrophotographic photoreceptor including an interlayer and a photosensitive layer in this order on a support, in which the interlayer contains a polymer of an electron transport material containing a non-hydrolyzable polymerizable functional group.

JP2003-345044A discloses an electrophotographic photoreceptor including an interlayer and a photosensitive layer in this order on a support, in which the interlayer contains a specific resin.

JP5147274B discloses an asymmetric imide compound having substituents with different structures.

JP4411232B discloses a method of producing an electrophotographic photoreceptor, including a step (i) of forming an interlayer on a conductive support by using a coating material for an interlayer that contains polynaphthyldiimide particles and a step (ii) of forming a photosensitive layer on the interlayer, in which the polynaphthyldiimide particles are particles of polynaphthyldiimide having a repeating unit that has a naphthyldiimide structure represented by General Formula (2).

JP2011-095665A discloses an electrophotographic photoreceptor including an interlayer and a photosensitive layer in this order on a conductive support, in which the interlayer contains a polyolefin resin and an organic electron transport material, the polyolefin resin is a specific polyolefin resin, and the organic electron transport material is a compound selected from the group consisting of an imide-based compound, a benzimidazole-based compound, a quinone-based compound, a cyclopentadienylidene-based compound, an azo-based compound, and derivatives thereof.

JP3958154B discloses an electrophotographic photoreceptor including an interlayer and a photosensitive layer in this order on a support, in which the photosensitive layer contains a charge generation substance and a charge transport substance, an electrostatic latent image is formed on a surface of the electrophotographic photoreceptor using a semiconductor laser, the interlayer contains a specific electron transport material, a volume resistivity of the interlayer in an environment of 30°C and 80% RH is 1×10¹² Ω·cm or greater, and a ratio (Rz/λ) of a ten-point average roughness (Rz) of the surface of the support on the photosensitive layer side to a wavelength (λ) of the semiconductor laser is 0.6 or greater and 2.5 or less.

WO 2005/092901 A1 discloses an electrophotographic photoreceptor comprising a conductive substrate, an undercoat layer and a photosensitive layer, wherein the undercoat layer comprises a binder resin and a product of perylene 3,4,9,10 tetracarboxylic acid dianhydride and diamine as electron transport material.

### SUMMARY OF THE INVENTION

In the electrophotographic photoreceptor including a conductive substrate, an undercoat layer, and a photosensitive layer of the related art, a method of adjusting charge maintainability by employing an undercoat layer that contains a binder resin and an electron transport material (such as the following electron transport material (A), (B), or (C)) is known. However, there has been a demand for development of an electrophotographic photoreceptor with more excellent charge maintainability.

An object of the present disclosure is to provide an electrophotographic photoreceptor with excellent charge maintainability as compared with an electrophotographic photoreceptor that employs an undercoat layer containing a binder resin and an electron transport material of the related art (such as the following electron transport material (A), (B), or (C)).

The present invention is defined in the appended claims. The following disclosure serves a better understanding of the present invention.

According to one of claims 1, 2 and 3, it is possible to provide an electrophotographic photoreceptor with excellent charge maintainability as compared with a case where an undercoat layer containing a binder resin and an electron transport material of the related art (such as the following electron transport material (A), (B), or (C)) is employed.

According to claim 4, it is possible to provide an electrophotographic photoreceptor with excellent charge maintainability as compared with a case where the average primary particle diameter of the electron transport material is greater than 1 µm.

According to claim 5, it is possible to provide an electrophotographic photoreceptor with excellent film forming properties and charge maintainability as compared with a case where the average primary particle diameter of the electron transport material is less than 0.03 µm or greater than 1 µm.

According to claim 6, it is possible to provide an electrophotographic photoreceptor with excellent film forming properties and charge maintainability as compared with a case where the content of the electron transport material is 70% by mass or greater with respect to the total solid content of the undercoat layer.

According to claim 7, it is possible to provide an electrophotographic photoreceptor with excellent charge maintainability as compared with a case where the undercoat layer has a thickness of less than 5 µm or greater than 15 µm.

According to claim 8, it is possible to provide an electrophotographic photoreceptor with excellent charge maintainability as compared with a case where the binder resin is a thermoplastic resin.

According to claim 9, it is possible to provide an electrophotographic photoreceptor with excellent charge maintainability as compared with a case where the thermosetting resin is nylon polyamide.

According to claim 10, it is possible to provide an electrophotographic photoreceptor with excellent charge maintainability as compared with a case where the content of the metal oxide in the undercoat layer is greater than 5% by mass with respect to the total solid content of the undercoat layer.

According to claim 11 or 12, it is possible to provide a process cartridge or an image forming apparatus including an electrophotographic photoreceptor with excellent charge maintainability as compared with a process cartridge or an image forming apparatus including an electrophotographic photoreceptor that employs an undercoat layer containing a binder resin and an electron transport material of the related art (such as the electron transport material (A), (B), or (C) described above).

### BRIEF DESCRIPTION OF THE DRAWINGS

Exemplary embodiment(s) of the present invention will be described in detail based on the following figures, wherein:
Fig. 1 is a schematic partial cross-sectional view showing an example of a layer configuration of an electrophotographic photoreceptor according to the present exemplary embodiment;
Fig. 2 is a schematic configuration view showing an example of an image forming apparatus according to the present exemplary embodiment; and
Fig. 3 is a schematic configuration view showing another example of the image forming apparatus according to the present exemplary embodiment.

### DETAILED DESCRIPTION OF THE INVENTION

Hereinafter, exemplary embodiments of the present disclosure will be described. The following descriptions and examples merely illustrate the exemplary embodiments, and do not limit the scope of the exemplary embodiments.

In the present specification, a numerical range shown using "to" indicates a range including numerical values described before and after "to" as a minimum value and a maximum value.

In a numerical range described in a stepwise manner in the present disclosure, an upper limit value or a lower limit value described in a certain numerical range may be replaced with an upper limit value or a lower limit value in another numerical range described in a stepwise manner. Further, in a numerical range described in the present disclosure, an upper limit value or a lower limit value described in the numerical range may be replaced with a value shown in Examples.

In the present disclosure, each component may include a plurality of kinds of substances corresponding to each component. In the present disclosure, in a case where a plurality of kinds of substances corresponding to each component in a composition are present, the amount of each component in the composition indicates the total amount of the plurality of kinds of substances present in the composition unless otherwise specified.

In the present disclosure, an electrophotographic photoreceptor is also simply referred to as a photoreceptor.

### <Electrophotographic Photoreceptor>

An electrophotographic photoreceptor according to the present exemplary embodiment includes a conductive substrate, an undercoat layer provided on the conductive substrate and containing a binder resin and an electron transport material represented by General Formula (P), a photosensitive layer provided on the undercoat layer.

In General Formula (P), R¹, R², R³, R⁴, R⁵, R⁶, R⁷, and R⁸ each independently represent a hydrogen atom, an alkyl group, an alkoxy group, an aralkyl group, an aryl group, an alkoxycarbonyl group, or a halogen atom.

The photoreceptor according to the present exemplary embodiment includes a conductive substrate, an undercoat layer disposed on the conductive substrate, and a photosensitive layer disposed on the undercoat layer.

Fig. 1 schematically shows an example of the layer configuration of the photoreceptor according to the present exemplary embodiment. A photoreceptor 7A shown in Fig. 1 has a structure in which an undercoat layer 1, a charge generation layer 2, and a charge transport layer 3 are laminated in this order on a conductive substrate 4. The charge generation layer 2 and the charge transport layer 3 constitute a photosensitive layer 5. The photoreceptor 7A may have a layer configuration in which a protective layer is further provided on the charge transport layer 3.

In the photoreceptor according to the present exemplary embodiment, the photosensitive layer may be a function separation type photosensitive layer in which the charge generation layer 2 and the charge transport layer 3 are separated as in the photoreceptor 7A shown in Fig. 1 or may be a single layer type photosensitive layer having a charge generation ability and a charge transport ability in place of the charge generation layer 2 and the charge transport layer 3.

The electrophotographic photoreceptor according to the present exemplary embodiment includes an undercoat layer containing a binder resin and an electron transport material represented by General Formula (P).

In order to improve the charge maintainability of the electrophotographic photoreceptor, the undercoat layer is required to have increased electron transport properties and lowered positive hole transport properties. For example, the above-described electron transport materials (A), (B), and (C) have been employed as the electron transport materials of the related art, and it has been found that since these materials have a high property of transporting electrons, but having a property of slightly moving positive holes, positive holes move due to the undercoat layer in a case where a voltage is applied to the electrophotographic photoreceptor, and thus charges are injected into a photosensitive layer. As a result, the positive hole blocking properties are not sufficient, the dark decay increases, and the charge maintainability tends to decrease.

Meanwhile, in the electrophotographic photoreceptor according to the present exemplary embodiment, the undercoat layer contains an electron transport material represented by General Formula (P) in addition to a binder resin. As a result of intensive examination conducted by the present inventors, it has been found that the electron transport material represented by General Formula (P) is a so-called perylenetetracarboxylic dianhydride, and has excellent electron transport properties as an electron transport material that is blended into the undercoat layer and low positive hole transport properties. As described above, the electrophotographic photoreceptor according to the present exemplary embodiment is considered to have excellent charge maintainability because the undercoat layer has excellent electron transport properties and reduces dark decay.

Hereinafter, each layer of the photoreceptor according to the present exemplary embodiment will be described in detail.

### [Undercoat Layer]

The undercoat layer contains a binder resin and an electron transport material represented by General Formula (P).

The undercoat layer may contain other materials in addition to the binder resin and the electron transport material represented by General Formula (P).

In General Formula (P), R¹, R², R³, R⁴, R⁵, R⁶, R⁷, and R⁸ each independently represent a hydrogen atom, an alkyl group, an alkoxy group, an aralkyl group, an aryl group, an alkoxycarbonyl group, or a halogen atom.

The electron transport material represented by General Formula (P) has excellent electron transport properties and low positive hole transport properties. Therefore, it is considered that in a case where the undercoat layer contains an electron transport material represented by General Formula (P), since the undercoat layer has excellent electron transport properties and reduces dark decay, the charge maintainability is excellent.

In General Formula (P), R¹, R², R³, R⁴, R⁵, R⁶, R⁷, and R⁸ each independently represent, for example, preferably a hydrogen atom or a halogen atom and more preferably a hydrogen atom.

It is considered that in a case where R¹ to R⁸ in General Formula (P) represent a hydrogen atom or a halogen atom (for example, more preferably a hydrogen atoms), the undercoat layer has more excellent electron transport properties and further reduces dark decay, and thus the charge maintainability is more excellent.

Examples of the alkyl group represented by R¹ to R⁸ in General Formula (P) include a substituted or unsubstituted alkyl group.

Examples of the unsubstituted alkyl group represented by R¹ to R⁸ in General Formula (P) include a linear alkyl group having 1 or more and 20 or less carbon atoms (for example, preferably 1 or more and 10 or less carbon atoms and more preferably 1 or more and 6 or less carbon atoms), a branched alkyl group having 3 or more and 20 or less carbon atoms (for example, preferably 3 or more and 10 or less carbon atoms), and a cyclic alkyl group having 3 or more and 20 or less carbon atoms (for example, preferably 3 or more and 10 or less carbon atoms).

Examples of the linear alkyl group having 1 or more and 20 or less carbon atoms include a methyl group, an ethyl group, an n-propyl group, an n-butyl group, an n-pentyl group, an n-hexyl group, an n-heptyl group, an n-octyl group, an n-nonyl group, an n-decyl group, an n-undecyl group, an n-dodecyl group, a tridecyl group, an n-tetradecyl group, an n-pentadecyl group, an n-heptadecyl group, an n-octadecyl group, an n-nonadecyl group, and an n-icosyl group.

Examples of the branched alkyl group having 3 or more and 20 or less carbon atoms include an isopropyl group, an isobutyl group, a sec-butyl group, a tert-butyl group, an isopentyl group, a neopentyl group, a tert-pentyl group, an isohexyl group, a sec-hexyl group, a tert-hexyl group, an isoheptyl group, a sec-heptyl group, a tert-heptyl group, an isooctyl group, a sec-octyl group, a tert-octyl group, an isononyl group, a sec-nonyl group, a tert-nonyl group, an isodecyl group, a sec-decyl group, a tert-decyl group, an isododecyl group, a sec-dodecyl group, a tert-dodecyl group, a tert-tetradecyl group, and a tert-pentadecyl group.

Examples of the cyclic alkyl group having 3 or more and 20 or less carbon atoms include a cyclopropyl group, a cyclobutyl group, a cyclopentyl group, a cyclohexyl group, a cycloheptyl group, a cyclooctyl group, a cyclononyl group, a cyclodecyl group, and polycyclic (for example, bicyclic, tricyclic, or spirocyclic) alkyl groups formed by these monocyclic alkyl groups being linked to each other.

Among these, for example, a linear alkyl group such as a methyl group or an ethyl group is preferable as the unsubstituted alkyl group.

Examples of the substituent in the alkyl group include an alkoxy group, a hydroxy group, a carboxy group, a nitro group, and a halogen atom (such as a fluorine atom, a bromine atom, or an iodine atom).

Examples of the alkoxy group that substitutes the hydrogen atom in the alkyl group include the same groups as the groups for the unsubstituted alkoxy group represented by R¹ to R⁸ in General Formula (P).

Examples of the alkoxy group represented by R¹ to R⁸ in General Formula (P) include a substituted or unsubstituted alkoxy group.

Examples of the unsubstituted alkoxy group represented by R¹ to R⁸ in General Formula (P) include a linear, branched, or cyclic alkoxy group having 1 or more and 10 or less carbon atoms (for example, preferably 1 or more and 6 or less carbon atoms and more preferably 1 or more and 4 or less carbon atoms).

Specific examples of the linear alkoxy group include a methoxy group, an ethoxy group, an n-propoxy group, an n-butoxy group, an n-pentyloxy group, an n-hexyloxy group, an n-heptyloxy group, an n-octyloxy group, an n-nonyloxy group, and an n-decyloxy group.

Specific examples of the branched alkoxy group include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, a tert-hexyloxy group, an isoheptyloxy group, a sec-heptyloxy group, a tert-heptyloxy group, an isooctyloxy group, a sec-octyloxy group, a tert-octyloxy group, an isononyloxy group, a sec-nonyloxy group, a tert-nonyloxy group, an isodecyloxy group, a sec-decyloxy group, and a tert-decyloxy group.

Specific examples of the cyclic alkoxy group include a cyclopropoxy group, a cyclobutoxy group, a cyclopentyloxy group, a cyclohexyloxy group, a cycloheptyloxy group, a cyclooctyloxy group, a cyclononyloxy group, and a cyclodecyloxy group.

Among these, for example, a linear alkoxy group is preferable as the unsubstituted alkoxy group.

Examples of the substituent in the alkoxy group include an aryl group, an alkoxycarbonyl group, an aryloxycarbonyl group, a hydroxyl group, a carboxy group, a nitro group, and a halogen atom (such as a fluorine atom, a bromine atom, or an iodine atom).

Examples of the aryl group that substitutes a hydrogen atom in the alkoxy group include the same groups as the groups for the unsubstituted aryl group represented by R¹ to R⁸ in General Formula (P).

Examples of the alkoxycarbonyl group that substitutes a hydrogen atom in the alkoxy group include the same groups as the groups for the unsubstituted alkoxycarbonyl group represented by R¹ to R⁸ in General Formula (P).

Examples of the aryloxycarbonyl group that substitutes a hydrogen atom in the alkoxy group include the same groups as the groups for the unsubstituted aryloxycarbonyl group represented by R¹ to R⁸ in General Formula (P).

Examples of the aralkyl group represented by R¹ to R⁸ in General Formula (P) include a substituted or unsubstituted aralkyl group.

In General Formula (P), as the unsubstituted aralkyl group represented by R¹ to R⁸, for example, an aralkyl group having 7 or more and 30 or less carbon atoms is preferable, an aralkyl group having 7 or more and 16 or less carbon atoms is more preferable, and an aralkyl group having 7 or more and 12 or less carbon atoms is still more preferable.

Examples of the unsubstituted aralkyl group having 7 or more and 30 or less carbon atoms include a benzyl group, a phenylethyl group, a phenylpropyl group, a 4-phenylbutyl group, a phenylpentyl group, a phenylhexyl group, a phenylheptyl group, a phenyloctyl group, a phenylnonyl group, a naphthylmethyl group, a naphthylethyl group, an anthracenylmethyl group, and a phenyl-cyclopentylmethyl group.

Examples of the substituent in the aralkyl group include an alkoxy group, an alkoxycarbonyl group, and a halogen atom (such as a fluorine atom, a bromine atom, or an iodine atom).

Examples of the alkoxy group that substitutes a hydrogen atom in the aralkyl group include the same groups as the groups for the unsubstituted alkoxy group represented by R¹ to R⁸ in General Formula (P).

Examples of the alkoxycarbonyl group that substitutes a hydrogen atom in the aralkyl group include the same groups as the groups for the unsubstituted alkoxycarbonyl group represented by R¹ to R⁸ in General Formula (P).

Examples of the aryl group represented by R¹ to R⁸ in General Formula (P) include a substituted or unsubstituted aryl group.

As the unsubstituted aryl group represented by R¹ to R⁸ in General Formula (P), for example, an aryl group having 6 or more and 30 or less carbon atoms is preferable, an aryl group having 6 or more and 14 or less carbon atoms is more preferable, and an aryl group having 6 or more and 10 or less carbon atoms is still more preferable.

Examples of the aryl group having 6 or more and 30 or less carbon atoms include a phenyl group, a biphenyl group, a 1-naphthyl group, a 2-naphthyl group, a 9-anthryl group, a 9-phenanthryl group, a 1-pyrenyl group, a 5-naphthacenyl group, a 1-indenyl group, a 2-azulenyl group, a 9-fluorenyl group, a biphenylenyl group, an indacenyl group, a fluoranthenyl group, an acenaphthylenyl group, an aceanthrylenyl group, a phenalenyl group, a fluorenyl group, an anthryl group, a bianthracenyl group, a teranthracenyl group, a quarter anthracenyl group, an anthraquinolyl group, a phenanthryl group, a triphenylenyl group, a pyrenyl group, a chrysenyl group, a naphthacenyl group, a preadenyl group, a picenyl group, a perylenyl group, a pentaphenyl group, a pentacenyl group, a tetraphenylenyl group, a hexaphenyl group, a hexacenyl group, a rubisenyl group, and a coronenyl group. Among these, for example, a phenyl group is preferable.

Examples of the substituent in the aryl group include an alkyl group, an alkoxy group, an alkoxycarbonyl group, an aryloxycarbonyl group, and a halogen atom (such as a fluorine atom, a bromine atom, or an iodine atom).

Examples of the alkyl group that substitutes a hydrogen atom in the aryl group include the same groups as the groups for the unsubstituted alkyl group represented by R¹ to R⁸ in General Formula (P).

Examples of the alkoxy group that substitutes a hydrogen atom in the aryl group include the same groups as the groups for the unsubstituted alkoxy group represented by R¹ to R⁸ in General Formula (P).

Examples of the alkoxycarbonyl group that substitutes a hydrogen atom in the aryl group include the same groups as the groups for the unsubstituted alkoxycarbonyl group represented by R¹ to R⁸ in General Formula (P).

Examples of the alkoxycarbonyl group represented by R¹ to R⁸ in General Formula (P) include a substituted or unsubstituted alkoxycarbonyl group.

The number of carbon atoms of the alkyl chain in the unsubstituted alkoxycarbonyl group represented by R¹ to R⁸ in General Formula (P) is, for example, preferably 1 or more and 20 or less, more preferably 1 or more and 15 or less, and still more preferably 1 or more and 10 or less.

Examples of the alkoxycarbonyl group having 1 or more and 20 or less carbon atoms in the alkyl chain include a methoxycarbonyl group, an ethoxycarbonyl group, a propoxycarbonyl group, an isopropoxycarbonyl group, an n-butoxycarbonyl group, a sec-butoxybutylcarbonyl group, a tert-butoxycarbonyl group, a pentaoxycarbonyl group, a hexaoxycarbonyl group, a heptaoxycarbonyl group, an octaoxycarbonyl group, a nonaoxycarbonyl group, a decaoxycarbonyl group, a dodecaoxycarbonyl group, a tridecaoxycarbonyl group, a tetradecaoxycarbonyl group, a pentadecaoxycarbonyl group, a hexadecaoxycarbonyl group, a heptadecaoxycarbonyl group, an octadecaoxycarbonyl group, a nonadecaoxycarbonyl group, and an icosaoxycarbonyl group.

Examples of the substituent in the alkoxycarbonyl group include an aryl group, a hydroxy group, and a halogen atom (such as a fluorine atom, a bromine atom, or an iodine atom).

Examples of the aryl group that substitutes a hydrogen atom in the alkoxycarbonyl group include the same groups as the groups for the unsubstituted aryl group represented by R¹ to R⁸ in General Formula (P).

Examples of the halogen atom represented by R¹ to R⁸ in General Formula (P) include a fluorine atom, a chlorine atom, a bromine atom, and an iodine atom.

Hereinafter, exemplary compounds of the electron transport material represented by General Formula (P) will be shown, but the present exemplary embodiment is not limited thereto. Further, the following exemplary compound numbers will be referred to as exemplary compounds (P-numbers) below.

| Example No. | Exemplary compound of electron transport material represented by General Formula (P) | Example No. | Exemplary compound of electron transport material represented by General Formula (P) |
|---|---|---|---|
| P-1 | | P-6 | |
| P-2 | | P-7 | |
| P-3 | | P-8 | |
| P-4 | | P-9 | |
| P-5 | | P-10 | |

| Example No. | Exemplary compound of electron transport material represented by General Formula (P) | Example No. | Exemplary compound of electron transport material represented by General Formula (P) |
|---|---|---|---|
| P-11 | | P-15 | |
| P-12 | | P-16 | |
| P-13 | | P-17 | |
| P-14 | | P-18 | |

The electron transport material represented by General Formula (P) has, for example, an average primary particle diameter of preferably 1 µm or less, more preferably 0.03 µm or greater and 1 µm or less, still more preferably 0.03 µm or greater and 0.8 µm or less, and particularly preferably 0.05 µm or greater and 0.7 µm or less.

In a case where the average primary particle diameter of the electron transport material represented by General Formula (P) is 1 µm or less, since the electron transport material is difficult to localize and is likely to be present with high dispersibility in the undercoat layer, the electron transport properties are likely to be more excellent and the positive hole transport properties are likely to be further decreased. In a case where the average primary particle diameter of the electron transport material is 0.03 µm or greater, since aggregation of the electron transport material is suppressed and the electron transport material is likely to be present with high dispersibility in the undercoat layer, the electron transport properties are likely to be more excellent and the positive hole transport properties are likely to be further decreased.

The average primary particle diameter of the electron transport material represented by General Formula (P) is determined as follows.

The electron transport material represented by General Formula (P) is specified by observing the laminated cross section of the undercoat layer of the electrophotographic photoreceptor in the thickness direction at a magnification of 100,000 times using a scanning electron microscope (SEM). Further, the particle diameters of any 10 particles present as the primary particles in the electron transport material represented by General Formula (P) that is present in the obtained SEM image are determined. An arithmetic average value of the obtained particle diameters is defined as the average primary particle diameter of the electron transport material.

The electron transport material represented by General Formula (P) has, for example, an aspect ratio of preferably 1.0 or greater and 5 or less, more preferably 1.1 or greater and 3 or less, and still more preferably 1.2 or greater and 2.5 or less.

In a case where the aspect ratio of the electron transport material represented by General Formula (P) is 2.5 or less, the electron transport material is likely to be present in the undercoat layer with high dispersibility, and thus the electron transport properties are likely to be more excellent and the positive hole transport properties are likely to be further decreased. In a case where the aspect ratio of the electron transport material is 1.0 or greater and 5 or less, the electron transport material is likely to be present in the undercoat layer with high dispersibility, and thus the electron transport properties are more excellent and the charge maintainability are maintained.

The aspect ratio of the electron transport material represented by General Formula (P) denotes a ratio (length of major axis/length of minor axis) of the length of the major axis of the electron transport material to the length of the minor axis of the electron transport material.

The length of the electron transport material in the major axis direction denotes the distance of the longest straight line formed by connecting one end portion and the other end portion of the electron transport material in the major axis direction. The length of the electron transport material in the minor axis direction denotes the distance of the longest straight line formed by connecting one end portion and the other end portion of the electron transport material in a direction orthogonal to the major axis.

The electron transport material represented by General Formula (P) is specified by removing the photosensitive layer (and the protective layer as necessary) from the electrophotographic photoreceptor and observing the undercoat layer using a field emission scanning electron microscope (JSM-6700F, manufactured by JEOL Ltd.) at a magnification of 3,000 to 100,000. The length of the major axis and the length of the minor axis are measured at any ten points of the electron transport material on the obtained micrograph, and each of the aspect ratios (length of major axis/length of minor axis) is determined. Further, the arithmetic average value of the obtained aspect ratios is defined as the aspect ratio of the electron transport material.

A method of adjusting the average primary particle diameter and the aspect ratio of the electron transport material represented by General Formula (P) to be in the above-described ranges is not particularly limited, and examples thereof include a method of pulverizing the electron transport material using a ball mill, a bead mill, a mortar, a sand mill, a kneader, an attritor or the like and a method of precipitating microcrystals by dissolving the electron transport material in fluoroacetic acid, sulfuric acid, or the like and bringing the mixture into contact with water or a poor solvent.

The undercoat layer may further contain other electron transport materials in addition to the electron transport materials represented by General Formula (P) within a range where the effects of the present disclosure are exhibited.

The proportion of the electron transport material represented by General Formula (P) in the total amount of the electron transport material in the undercoat layer is, for example, preferably 80% by mass or greater and 100% by mass or less, more preferably 90% by mass or greater and 100% by mass or less, and still more preferably 95% by mass or greater and 100% by mass or less.

The content of the electron transport material represented by General Formula (P) is, for example, preferably less than 70% by mass, more preferably 45% by mass or greater and less than 60% by mass, and still more preferably 50% by mass or greater and less than 60% by mass with respect to the total solid content of the undercoat layer.

In the related art, from the viewpoint of ensuring both the electron mobility and the charge maintainability, the content of the electron transport material represented by General Formula (P) in the undercoat layer is, for example, preferably 70% by mass or greater with respect to the total solid content of the undercoat layer. Meanwhile, in the present exemplary embodiment, since the undercoat layer contains the electron transport material represented by General Formula (P), which has excellent electron transport properties and low positive hole transport properties, both the electron mobility and the charge maintainability can be achieved even when the content of the electron transport material is less than 70% by mass.

The content of the electron transport material represented by General Formula (P) may be 60% by mass or greater and 60% by mass or greater and 70% by mass or less with respect to the total solid content of the undercoat layer. In a case where the content of the electron transport material is 70% by mass or less, degradation of the film quality, a decrease in the film forming properties, and occurrence of surface roughness on the undercoat layer are suppressed, and thus the charge maintainability is more excellent. Meanwhile, in a case where the content of the electron transport material is 60% by mass or greater, the electron transport ability is sufficient, and the charge maintainability is more excellent.

Examples of the binder resin include known polymer compounds such as an acetal resin (such as polyvinyl butyral), a polyvinyl alcohol resin, a polyvinyl acetal resin, a casein resin, a diallyl phthalate resin, a polyamide resin, a nylon resin, a nylon polyamide resin, a cellulose resin, gelatin, a urethane resin, a melamine resin, a benzoguanamine resin (such as a methylated benzoguanamine resin), a polyester resin, an unsaturated polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a urea resin, a phenol resin (such as a resol type phenol resin), a phenol-formaldehyde resin, an alkyd resin, and an epoxy resin; a zirconium chelate compound; a titanium chelate compound; an aluminum chelate compound; a titanium alkoxide compound; an organic titanium compound; and known materials such as a silane coupling agent.

Examples of the binder resin used for the undercoat layer include a charge-transporting resin containing a charge-transporting group, and a conductive resin (such as polyaniline). The binder resin may be used alone or in combination of two or more kinds thereof. In a case where the binder resin is used in combination of two or more kinds thereof, the mixing ratio thereof is set as necessary.

In the present specification, the concept of the binder resin includes a resin obtained by a reaction between the resin described above and a curing agent and a resin obtained by a reaction of a curing agent.

In the present specification, the resin obtained by a reaction between a urethane resin and a curing agent will be referred to as "curing type urethane resin" for convenience.

The binder resin may be any of a thermoplastic resin or a thermosetting resin, and for example, a thermosetting resin is preferable. For example, from the viewpoint that dissolution or swelling of a film does not occur in the formation of a coating film of an upper layer, it is preferable that the binder resin is a thermosetting resin.

Among these, as the binder resin used in the undercoat layer, for example, a resin that is insoluble in the coating solvent of the upper layer is preferable, a resin obtained by a reaction of a curing agent and at least one resin selected from the group consisting of a diallyl phthalate resin, a polyamide resin, a nylon resin, a urethane resin, a melamine resin, a benzoguanamine resin, and a phenol resin is preferable, and it is more preferable that the binder resin includes at least one resin selected from the group consisting of a urethane resin, a melamine resin, and a benzoguanamine resin. In a case where the binder resin includes at least one resin selected from the above-described group, the positive hole blocking properties are high and the charge maintainability is excellent.

The proportion of at least one resin selected from the group consisting of a urethane resin, a melamine resin, and a benzoguanamine resin in the total amount of the binder resin in the undercoat layer is, for example, preferably 80% by mass or greater and 100% by mass or less, more preferably 90% by mass or greater and 100% by mass or less, and still more preferably 95% by mass or greater and 100% by mass or less.

The undercoat layer may further contain inorganic particles.

Examples of the inorganic particles include inorganic particles having a powder resistance (volume resistivity) of 10² Ω·cm or greater and 10¹¹ Ω·cm or less.

Among these, as the inorganic particles having the above-described resistance value, for example, metal oxide particles such as tin oxide particles, titanium oxide particles, zinc oxide particles, and zirconium oxide particles may be used, and zinc oxide particles are particularly preferable.

The specific surface area of the inorganic particles measured by the BET method may be, for example, 10 m²/g or greater. In a case where the specific surface area thereof is 10 m²/g or greater, degradation of the charging properties tends to be suppressed.

The volume average particle diameter of the inorganic particles may be, for example, 50 nm or greater and 2,000 nm or less (for example, preferably 60 nm or greater and 1,000 nm or less).

The content of the inorganic particles is, for example, preferably 0% by mass or greater and 80% by mass or less and more preferably 0% by mass or greater and 70% by mass or less with respect to the total solid content of the undercoat layer.

The inorganic particles may be subjected to a surface treatment. As the inorganic particles, inorganic particles subjected to different surface treatments or inorganic particles having different particle diameters may be used in the form of a mixture of two or more kinds thereof.

Examples of the surface treatment agent include a silane coupling agent, a titanate-based coupling agent, an aluminum-based coupling agent, and a surfactant. In particular, for example, a silane coupling agent is preferable, and a silane coupling agent containing an amino group is more preferable.

Examples of the silane coupling agent containing an amino group include 3-aminopropyltriethoxysilane, N-2-(aminoethyl)-3-aminopropyltrimethoxysilane, N-2-(aminoethyl)-3-aminopropylmethyldimethoxysilane, and N,N-bis(2-hydroxyethyl)-3-aminopropyltriethoxysilane, but are not limited thereto.

The silane coupling agent may be used in the form of a mixture of two or more kinds thereof. For example, a silane coupling agent containing an amino group and another silane coupling agent may be used in combination. Examples of other silane coupling agents include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl)-3-aminopropyltriethoxysilane, and 3-chloropropyltrimethoxysilane, but are not limited thereto.

The surface treatment method using a surface treatment agent may be any method as long as the method is a known method, and any of a dry method or a wet method may be used.

The treatment amount of the surface treatment agent is, for example, preferably 0.5% by mass or greater and 10% by mass or less with respect to the amount of the inorganic particles.

The dry method is, for example, a method of attaching the surface treatment agent to the surface of the inorganic particles by directly adding the surface treatment agent to the inorganic particles or adding the surface treatment agent, which has been dissolved in an organic solvent, dropwise to the inorganic particles while being stirred with a mixer having a large shearing force and spraying the mixture together with dry air or nitrogen gas. The surface treatment agent may be added dropwise or sprayed, for example, at a temperature lower than or equal to the boiling point of the solvent. After the dropwise addition or the spraying of the surface treatment agent, the surface treatment agent may be further baked at 100°C or higher. The baking is not particularly limited as long as the temperature and the time are adjusted such that the electrophotographic characteristics can be obtained.

The wet method is, for example, a method of attaching the surface treatment agent to the surface of inorganic particles by adding the surface treatment agent to the inorganic particles while dispersing the inorganic particles in a solvent by performing stirring or using ultrasonic waves, a sand mill, an attritor, or a ball mill, stirring or dispersing the mixture, and removing the solvent. The solvent removing method is carried out by, for example, filtration or distillation so that the solvent is distilled off. After removal of the solvent, the mixture may be further baked at 100°C or higher. The baking is not particularly limited as long as the temperature and the time are adjusted such that the electrophotographic characteristics can be obtained. In the wet method, the moisture contained in the inorganic particles may be removed before the surface treatment agent is added, and examples thereof include a method of removing the moisture while stirring and heating the moisture in a solvent and a method of removing the moisture by azeotropically boiling the moisture with a solvent.

The undercoat layer may further contain various additives for improving the electrical properties, the environmental stability, and the image quality.

Examples of the additives include known materials, for example, an electrontransport material such as a polycyclic condensed material or an azo-based material, a zirconium chelate compound, a titanium chelate compound, an aluminum chelate compound, a titanium alkoxide compound, an organic titanium compound, and a silane coupling agent. The silane coupling agent is used for a surface treatment of the inorganic particles as described above, but may be further added to the undercoat layer as an additive.

Examples of the silane coupling agent serving as an additive include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl)-3-aminopropyltriethoxysilane, and 3-chloropropyltrimethoxysilane.

Examples of the zirconium chelate compound include zirconium butoxide, ethyl zirconium acetoacetate, zirconium triethanolamine, acetylacetonate zirconium butoxide, ethyl zirconium butoxide acetoacetate, zirconium acetate, zirconium oxalate, zirconium lactate, zirconium phosphonate, zirconium octanoate, zirconium naphthenate, zirconium laurate, zirconium stearate, zirconium isostearate, zirconium butoxide methacrylate, stearate zirconium butoxide, and isostearate zirconium butoxide.

Examples of the titanium chelate compound include tetraisopropyl titanate, tetranormal butyl titanate, a butyl titanate dimer, tetra(2-ethylhexyl) titanate, titanium acetylacetonate, polytitanium acetylacetonate, titanium octylene glycolate, titanium lactate ammonium salt, titanium lactate, titanium lactate ethyl ester, titanium triethanol aminate, and polyhydroxy titanium stearate.

Examples of the aluminum chelate compound include aluminum isopropylate, monobutoxyaluminum diisopropylate, aluminum butyrate, diethylacetoacetate aluminum diisopropylate, and aluminum tris(ethylacetoacetate).

These additives may be used alone or in the form of a mixture or a polycondensate of a plurality of compounds.

The volume resistivity of the undercoat layer is, for example, preferably 1×10¹⁰ Ω·cm or greater and 1×10¹² Ω·cm or less.

The undercoat layer may have, for example, a Vickers hardness of 35 or greater.

The surface roughness (ten-point average roughness) of the undercoat layer may be adjusted, for example, to 1/2 from 1/(4n) (n represents a refractive index of an upper layer) of a laser wavelength λ for exposure to be used to suppress moire fringes.

Resin particles or the like may be added to the undercoat layer to adjust the surface roughness. Examples of the resin particles include silicone resin particles and crosslinked polymethyl methacrylate resin particles. Further, the surface of the undercoat layer may be polished to adjust the surface roughness. Examples of the polishing method include buff polishing, a sandblast treatment, wet honing, and a grinding treatment.

### - Method of Forming Undercoat Layer -

The formation of the undercoat layer is not particularly limited, and a known forming method is used. For example, a coating film of a coating solution for forming an undercoat layer in which the above-described components are added to a solvent is formed, and the coating film is dried and, as necessary, heated.

Examples of the solvent for preparing the coating solution for forming an undercoat layer include known organic solvents such as an alcohol-based solvent, an aromatic hydrocarbon solvent, a halogenated hydrocarbon solvent, a ketone-based solvent, a ketone alcohol-based solvent, an ether-based solvent, and an ester-based solvent.

Specific examples of these solvents include typical organic solvents such as methanol, ethanol, n-propanol, iso-propanol, n-butanol, benzyl alcohol, methyl cellosolve, ethyl cellosolve, acetone, methyl ethyl ketone, cyclohexanone, methyl acetate, ethyl acetate, n-butyl acetate, dioxane, tetrahydrofuran, methylene chloride, chloroform, chlorobenzene, and toluene.

Examples of the method of dispersing the inorganic particles when preparing the coating solution for forming an undercoat layer include known methods such as a roll mill, a ball mill, a vibration ball mill, an attritor, a sand mill, a colloid mill, and a paint shaker.

Since the electron transport material (particularly, the electron transport material represented by General Formula (P)) is unlikely to be dissolved in an organic solvent, for example, it is desirable that the electron transport material is dispersed in an organic solvent. Examples of a dispersing method include known methods such as a roll mill, a ball mill, a vibration ball mill, an attritor, a sand mill, a colloid mill, and a paint shaker. In a case where the metal oxide particles are blended into the undercoat layer, for example, it is desirable that the metal oxide particles are dispersed in an organic solvent by the same dispersing method.

Examples of the method of coating the conductive substrate with the coating solution for forming an undercoat layer include typical coating methods such as a blade coating method, a wire bar coating method, a spray coating method, a dip coating method, a bead coating method, an air knife coating method, and a curtain coating method.

The content of the metal oxide in the undercoat layer is, for example, preferably 5% by mass or less, more preferably 3% by mass or less, and still more preferably 0% by mass (that is, the undercoat layer contains no metal oxide) or 2% by mass or less with respect to the total solid content of the undercoat layer.

In general, the metal oxide tends to have low resistance. Therefore, in a case where the content of the metal oxide in the undercoat layer is 5% by mass or less, degradation of the charging properties due to a decrease in the resistance of the undercoat layer is suppressed. Further, from the viewpoint of production aiming at reducing the environmental load, for example, it is preferable that the content of the metal oxide is decreased.

From the viewpoint that the charge maintainability is more excellent, the thickness of the undercoat layer is, for example, preferably 5 µm or greater and 15 µm or less, more preferably 7 µm or greater and 14 µm or less, and still more preferably 8 µm or greater and 13 µm or less.

The thickness of the undercoat layer may be 15 µm or greater or 20 µm or greater and 50 µm or less.

Since an organic pigment-based electron transport material of the related art considerably has positive hole transport properties in addition to electron transport properties, injection of positive holes from the conductive substrate or injection of positive holes into the charge generation layer which is the upper layer are likely to occur during charging of the electrophotographic photoreceptor in a case where the organic pigment-based electron transport material is used in the undercoat layer, and problems such as degradation of the charging properties and an increase in dark decay after charging and an adverse effect on the image quality due to degradation of the charge maintainability are likely to occur. This tendency tends to increase as the thickness of the undercoat layer increases. Therefore, the undercoat layer is required to have a small thickness (for example, 5 µm or less) in actual use.

However, in a case where the undercoat layer is thin and foreign matter from the outside (such as a toner carrier or a wear piece of a plastic component), particularly needle-like foreign matter such as carbon fibers adheres to the surface of the photoreceptor during image formation, the foreign matter may be stuck into the surface of the photoreceptor due to the contact pressure with the intermediate transfer member and leakage current may occur. On the contrary, in the present exemplary embodiment, since the undercoat layer contains the electron transport material represented by General Formula (P), which has excellent electron transport properties, low positive hole transport properties, and satisfactory charge maintainability, the film thickness of the undercoat layer can be made larger (for example, 5 µm or greater) than the film thickness of the undercoat layer formed of an organic pigment of the related art as a main agent. Therefore, it is considered that even in a case where foreign matter is stuck into a region from the surface of the electrophotographic photoreceptor to the undercoat layer, the leakage current is unlikely to occur, and thus the charge maintainability is excellent.

In a case where the thickness of the undercoat layer is at least 15 µm or less, since sufficient electron transport properties are exhibited within the time of the electrophotographic photoreceptor process and the resistance in the bulk of the undercoat layer can be maintained high, the resistance to leakage caused by foreign matter and the charge maintainability during a long-term cycle can be maintained.

### [Conductive Substrate]

Examples of the conductive substrate include metal plates containing metals (such as aluminum, copper, zinc, chromium, nickel, molybdenum, vanadium, indium, gold, and platinum) or alloys (such as stainless steel), metal drums, metal belts, and the like. Further, examples of the conductive substrate include paper, a resin film, a belt, and the like obtained by being coated, vapor-deposited or laminated with a conductive compound (such as a conductive polymer or indium oxide), a metal (such as aluminum, palladium, or gold) or an alloy. Here, the term "conductive" denotes that the volume resistivity is less than 10¹³ Ω·cm.

In a case where the electrophotographic photoreceptor is used in a laser printer, for example, it is preferable that the surface of the conductive substrate is roughened such that a centerline average roughness Ra thereof is 0.04 µm or greater and 0.5 µm or less for the purpose of suppressing interference fringes from occurring in a case of irradiation with laser beams. Further, in a case where incoherent light is used as a light source, roughening of the surface to prevent interference fringes is not particularly necessary, and it is appropriate for longer life because occurrence of defects due to the roughness of the surface of the conductive substrate is suppressed.

Examples of the roughening method include wet honing performed by suspending an abrasive in water and spraying the suspension to the conductive substrate, centerless grinding performed by pressure-welding the conductive substrate against a rotating grindstone and continuously grinding the conductive substrate, and an anodizing treatment.

Examples of the roughening method also include a method of dispersing conductive or semi-conductive powder in a resin without roughening the surface of the conductive substrate to form a layer on the surface of the conductive substrate, and performing roughening using the particles dispersed in the layer.

The roughening treatment performed by anodization is a treatment of forming an oxide film on the surface of the conductive substrate by carrying out anodization in an electrolytic solution using a conductive substrate made of a metal (for example, aluminum) as an anode. Examples of the electrolytic solution include a sulfuric acid solution and an oxalic acid solution. However, a porous anodized film formed by anodization is chemically active in a natural state, is easily contaminated, and has a large resistance fluctuation depending on the environment. Therefore, for example, it is preferable that a sealing treatment is performed on the porous anodized film so that the micropores of the oxide film are closed by volume expansion due to a hydration reaction in pressurized steam or boiling water (a metal salt such as nickel may be added thereto) for a change into a more stable a hydrous oxide.

The film thickness of the anodized film is, for example, preferably 0.3 µm or greater and 15 µm or less. In a case where the film thickness is in the above-described range, the barrier properties against injection tend to be exhibited, and an increase in the residual potential due to repeated use tends to be suppressed.

The conductive substrate may be subjected to a treatment with an acidic treatment liquid or a boehmite treatment.

The treatment with an acidic treatment liquid is carried out, for example, as follows. First, an acidic treatment liquid containing phosphoric acid, chromic acid, and hydrofluoric acid is prepared. In the blending ratio of phosphoric acid, chromic acid, and hydrofluoric acid to the acidic treatment liquid, for example, the concentration of the phosphoric acid is 10% by mass or greater and 11% by mass or less, the concentration of the chromic acid is 3% by mass or greater and 5% by mass or less, and the concentration of the hydrofluoric acid is 0.5% by mass or greater and 2% by mass or less, and the concentration of all these acids may be 13.5% by mass or greater and 18% by mass or less. The treatment temperature is, for example, preferably 42°C or higher and 48°C or lower. The film thickness of the coating film is, for example, preferably 0.3 µm or greater and 15 µm or less.

The boehmite treatment is carried out, for example, by dipping the conductive substrate in pure water at 90°C or higher and 100°C or lower for 5 minutes to 60 minutes or by bringing the conductive substrate into contact with heated steam at 90°C or higher and 120°C or lower for 5 minutes to 60 minutes. The film thickness of the coating film is, for example, preferably 0.1 µm or greater and 5 µm or less. This coating film may be further subjected to the anodizing treatment using an electrolytic solution having low film solubility, such as adipic acid, boric acid, a borate, a phosphate, a phthalate, a maleate, a benzoate, a tartrate, or a citrate.

### (Interlayer)

Although not shown in the figures, an interlayer may be further provided between the undercoat layer and the photosensitive layer.

The interlayer is, for example, a layer containing a resin. Examples of the resin used for the interlayer include a polymer compound, for example, an acetal resin (such as polyvinyl butyral), a polyvinyl alcohol resin, a polyvinyl acetal resin, a casein resin, a polyamide resin, a cellulose resin, gelatin, a polyurethane resin, a polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a phenol-formaldehyde resin, or a melamine resin.

The interlayer may be a layer containing an organometallic compound. Examples of the organometallic compound used for the interlayer include an organometallic compound containing metal atoms such as zirconium, titanium, aluminum, manganese, and silicon.

The compounds used for the interlayer may be used alone or in the form of a mixture or a polycondensate of a plurality of compounds.

Among these, it is preferable that the interlayer is, for example, a layer containing an organometallic compound having a zirconium atom or a silicon atom.

The formation of the interlayer is not particularly limited, and a known forming method is used. For example, a coating film of a coating solution for forming an interlayer in which the above-described components are added to a solvent is formed, and the coating film is dried and, as necessary, heated.

Examples of the coating method of forming the interlayer include typical methods such as a dip coating method, a push-up coating method, a wire bar coating method, a spray coating method, a blade coating method, an air knife coating method, and a curtain coating method.

The film thickness of the interlayer is set to be, for example, preferably in a range of 0.1 µm or greater and 3 µm or less. Further, the interlayer may be used as the undercoat layer.

### (Charge Generation Layer)

The charge generation layer is, for example, a layer containing a charge generation material and a binder resin. Further, the charge generation layer may be a deposition layer of the charge generation material. The deposition layer of the charge generation material is, for example, preferable in a case where an incoherent light source such as a light emitting diode (LED) or an organic electro-luminescence (EL) image array is used.

Examples of the charge generation material include an azo pigment such as bisazo or trisazo; a fused ring aromatic pigment such as dibromoanthanthrone; a perylene pigment; a pyrrolopyrrole pigment; a phthalocyanine pigment; zinc oxide; and trigonal selenium.

Among these, for example, a metal phthalocyanine pigment or a metal-free phthalocyanine pigment is preferably used as the charge generation material in order to deal with laser exposure in a near infrared region. Specifically, for example, hydroxygallium phthalocyanine; chlorogallium phthalocyanine; dichlorotin phthalocyanine; and titanyl phthalocyanine are more preferable.

On the other hand, for example, a fused ring aromatic pigment such as dibromoanthanthrone; a thioindigo-based pigment; a porphyrazine compound; zinc oxide; trigonal selenium; or a bisazo pigment is preferable as the charge generation material in order to deal with laser exposure in a near ultraviolet region.

The above-described charge generation material may also be used even in a case where an incoherent light source such as an LED or an organic EL image array having a center wavelength of light emission at 450 nm or greater and 780 nm or less is used.

Meanwhile, in a case where an n-type semiconductor such as a fused ring aromatic pigment, a perylene pigment, or an azo pigment is used as the charge generation material, a dark current is unlikely to be generated, and image defects referred to as black spots can be suppressed even in a case where a thin film is used as the photosensitive layer.

Further, the n-type is determined by the polarity of the flowing photocurrent using a typically used time-of-flight method, and a material in which electrons more easily flow as carriers than positive holes is determined as the n-type.

The binder resin used for the charge generation layer is selected from a wide range of insulating resins, and the binder resin may be selected from organic photoconductive polymers such as poly-N-vinylcarbazole, polyvinyl anthracene, polyvinylpyrene, and polysilane.

Examples of the binder resin include a polyvinyl butyral resin, a polyarylate resin (a polycondensate of bisphenols and aromatic divalent carboxylic acid), a polycarbonate resin, a polyester resin, a phenoxy resin, a vinyl chloride-vinyl acetate copolymer, a polyamide resin, an acrylic resin, a polyacrylamide resin, a polyvinylpyridine resin, a cellulose resin, a urethane resin, an epoxy resin, casein, a polyvinyl alcohol resin, and a polyvinylpyrrolidone resin. Here, the term "insulating" denotes that the volume resistivity is 10¹³ Ω·cm or greater.

These binder resins may be used alone or in the form of a mixture of two or more kinds thereof.

Further, the blending ratio between the charge generation material and the binder resin is, for example, preferably in a range of 10:1 to 1:10 in terms of the mass ratio.

The charge generation layer may also contain other known additives.

The formation of the charge generation layer is not particularly limited, and a known forming method is used. For example, a coating film of a coating solution for forming a charge generation layer in which the above-described components are added to a solvent is formed, and the coating film is dried and, as necessary, heated. Further, the charge generation layer may be formed by vapor deposition of the charge generation material. The formation of the charge generation layer by vapor deposition is, for example, particularly appropriate in a case where a fused ring aromatic pigment or a perylene pigment is used as the charge generation material.

Examples of the solvent for preparing the coating solution for forming a charge generation layer include methanol, ethanol, n-propanol, n-butanol, benzyl alcohol, methyl cellosolve, ethyl cellosolve, acetone, methyl ethyl ketone, cyclohexanone, methyl acetate, n-butyl acetate, dioxane, tetrahydrofuran, methylene chloride, chloroform, chlorobenzene, and toluene. These solvents are used alone or in the form of a mixture of two or more kinds thereof.

As a method of dispersing particles (for example, the charge generation material) in the coating solution for forming a charge generation layer, for example, a media disperser such as a ball mill, a vibration ball mill, an attritor, a sand mill, or a horizontal sand mill, or a medialess disperser such as a stirrer, an ultrasonic disperser, a roll mill, or a high-pressure homogenizer is used. Examples of the high-pressure homogenizer include a collision type high-pressure homogenizer in which a dispersion liquid is dispersed by a liquid-liquid collision or a liquid-wall collision in a high-pressure state, and a penetration type high-pressure homogenizer in which a dispersion liquid is dispersed by causing the liquid to penetrate through a micro-flow path in a high-pressure state.

During the dispersion, it is effective to set the average particle diameter of the charge generation material in the coating solution for forming a charge generation layer to 0.5 µm or less, for example, preferably 0.3 µm or less, and more preferably 0.15 µm or less.

Examples of the method of coating the undercoat layer (or the interlayer) with the coating solution for forming a charge generation layer include typical methods such as a blade coating method, a wire bar coating method, a spray coating method, a dip coating method, a bead coating method, an air knife coating method, and a curtain coating method.

The film thickness of the charge generation layer is set to be, for example, in a range of preferably 0.1 µm or greater and 5.0 µm or less and more preferably in a range of 0.2 µm or greater and 2.0 µm or less.

### (Charge Transport Layer)

The charge transport layer is, for example, a layer containing a charge transport material and a binder resin. The charge transport layer may be a layer containing a polymer charge transport material.

Examples of the charge transport material include a quinone-based compound such as p-benzoquinone, chloranil, bromanil, or anthraquinone; a tetracyanoquinodimethane-based compound; a fluorenone compound such as 2,4,7-trinitrofluorenone; a xanthone-based compound; a benzophenone-based compound; a cyanovinyl-based compound; and an electron-transporting compound such as an ethylene-based compound. Examples of the charge transport material include a positive hole-transporting compound such as a triarylamine-based compound, a benzidine-based compound, an arylalkane-based compound, an aryl-substituted ethylene-based compound, a stilbene-based compound, an anthracene-based compound, or a hydrazone-based compound. These charge transport materials may be used alone or in combination of two or more kinds thereof, but are not limited thereto.

From the viewpoint of the charge mobility, for example, a triarylamine derivative represented by Structural Formula (a-1) or a benzidine derivative represented by Structural Formula (a-2) is preferable as the charge transport material.

In Structural Formula (a-1), Ar^{T1}, Ar^{T2}, and Ar^{T3} each independently represent a substituted or unsubstituted aryl group, -C₆H₄-C(R^{T4})=C(R^{T5})(R^{T6}), or -C₆H₄-CH=CH-CH=C(R^{T7})(R^{T8}). R^{T4}, R^{T5}, R^{T6}, R^{T7}, and R^{T8} each independently represent a hydrogen atom, a substituted or unsubstituted alkyl group, or a substituted or unsubstituted aryl group.

Examples of the substituent of each group described above include a halogen atom, an alkyl group having 1 or more and 5 or less carbon atoms, and an alkoxy group having 1 or more and 5 or less carbon atoms. Further, examples of the substituent of each group described above include a substituted amino group substituted with an alkyl group having 1 or more and 3 or less carbon atoms.

In Structural Formula (a-2), R^{T91} and R^{T92} each independently represent a hydrogen atom, a halogen atom, an alkyl group having 1 or more and 5 or less carbon atoms, or an alkoxy group having 1 or more and 5 or less carbon atoms. R^{T101}, R^{T102}, R^{T111}, and R^{T112} each independently represent a halogen atom, an alkyl group having 1 or more and 5 or less carbon atoms, an alkoxy group having 1 or more and 5 or less carbon atoms, an amino group substituted with an alkyl group having 1 or more and 2 or less carbon atoms, a substituted or unsubstituted aryl group, -C(R^{T12})=C(R^{T13})(R^{T14}), or -CH=CH-CH=C(R^{T15})(R^{T16}), and R^{T12}, R^{T13}, R^{T14}, R^{T15}, and R^{T16} each independently represent a hydrogen atom, a substituted or unsubstituted alkyl group, or a substituted or unsubstituted aryl group. Tm1, Tm2, Tn1, and Tn2 each independently represent an integer of 0 or greater and 2 or less.

Examples of the substituent of each group described above include a halogen atom, an alkyl group having 1 or more and 5 or less carbon atoms, and an alkoxy group having 1 or more and 5 or less carbon atoms. Further, examples of the substituent of each group described above include a substituted amino group substituted with an alkyl group having 1 or more and 3 or less carbon atoms.

Here, among the triarylamine derivative represented by Structural Formula (a-1) and the benzidine derivative represented by Structural Formula (a-2), for example, a triarylamine derivative having "-C₆H₄-CH=CH-CH=C(R^{T7})(R^{T8})" and a benzidine derivative having "-CH=CH-CH=C(R^{T15})(R^{T16})" are particularly preferable from the viewpoint of the charge mobility.

As the polymer charge transport material, known materials having charge transport properties, such as poly-N-vinylcarbazole and polysilane, can be used. Particularly, for example, a polyester-based polymer charge transport material is particularly preferable. Further, the polymer charge transport material may be used alone or in combination of binder resins.

Examples of the binder resin used for the charge transport layer include a polycarbonate resin, a polyester resin, a polyarylate resin, a methacrylic resin, an acrylic resin, a polyvinyl chloride resin, a polyvinylidene chloride resin, a polystyrene resin, a polyvinyl acetate resin, a styrene-butadiene copolymer, a vinylidene chloride-acrylonitrile copolymer, a vinyl chloride-vinyl acetate copolymer, a vinyl chloride-vinyl acetate-maleic anhydride copolymer, a silicone resin, a silicone alkyd resin, a phenol-formaldehyde resin, a styrene-alkyd resin, poly-N-vinylcarbazole, and polysilane. Among these, for example, a polycarbonate resin or a polyarylate resin is preferable as the binder resin. These binder resins may be used alone or in combination of two or more kinds thereof.

Further, the blending ratio between the charge transport material and the binder resin is, for example, preferably in a range of 10:1 to 1:5 in terms of the mass ratio.

The charge transport layer may also contain other known additives.

The formation of the charge transport layer is not particularly limited, and a known forming method is used. For example, a coating film of a coating solution for forming a charge transport layer in which the above-described components are added to a solvent is formed, and the coating film is dried and, as necessary, heated.

Examples of the solvent for preparing the coating solution for forming a charge transport layer include typical organic solvents, for example, aromatic hydrocarbons such as benzene, toluene, xylene, and chlorobenzene; ketones such as acetone and 2-butanone; halogenated aliphatic hydrocarbons such as methylene chloride, chloroform, and ethylene chloride; and cyclic or linear ethers such as tetrahydrofuran and ethyl ether. These solvents are used alone or in the form of a mixture of two or more kinds thereof.

Examples of the coating method of coating the charge generation layer with the coating solution for forming a charge transport layer include typical methods such as a blade coating method, a wire bar coating method, a spray coating method, a dip coating method, a bead coating method, an air knife coating method, and a curtain coating method.

The film thickness of the charge transport layer is set to be, for example, preferably in a range of 5 µm or greater and 50 µm or less and more preferably in a range of 10 µm or greater and 30 µm or less.

### (Protective Layer)

A protective layer is provided on the photosensitive layer as necessary. The protective layer is provided, for example, for the purpose of preventing a chemical change in the photosensitive layer during charging and further improving the mechanical strength of the photosensitive layer.

Therefore, for example, a layer formed of a cured film (crosslinked film) may be applied to the protective layer. Examples of these layers include the layers described in the items 1) and 2) below.
1) A layer formed of a cured film of a composition containing a reactive group-containing charge transport material having a reactive group and a charge-transporting skeleton in an identical molecule (that is, a layer containing a polymer or a crosslinked body of the reactive group-containing charge transport material)
2) A layer formed of a cured film of a composition containing a non-reactive charge transport material and a reactive group-containing non-charge transport material containing a reactive group without having a charge-transporting skeleton (that is, a layer containing the non-reactive charge transport material and a polymer or crosslinked body of the reactive group-containing non-charge transport material)

Examples of the reactive group of the reactive group-containing charge transport material include known reactive groups such as a chain polymerizable group, an epoxy group, - OH, -OR [here, R represents an alkyl group], -NH₂, -SH, -COOH, and -SiR^{Q1}_{3-Qn}(OR^{Q2} )_{Qn} [here, R^{Q1} represents a hydrogen atom, an alkyl group, or a substituted or unsubstituted aryl group, R^{Q2} represents a hydrogen atom, an alkyl group, or a trialkylsilyl group, and Qn represents an integer of 1 to 3].

The chain polymerizable group is not particularly limited as long as the group is a functional group capable of radical polymerization and is, for example, a functional group containing a group having at least a carbon double bond. Specific examples thereof include a vinyl group, a vinyl ether group, a vinyl thioether group, a styryl group (vinylphenyl group), an acryloyl group, a methacryloyl group, and a group containing at least one selected from derivatives thereof. Among these, from the viewpoint that the reactivity is excellent, for example, a vinyl group, a styryl group (vinylphenyl group), an acryloyl group, a methacryloyl group, and a group containing at least one selected from derivatives thereof are preferable as the chain polymerizable group.

The charge-transporting skeleton of the reactive group-containing charge transport material is not particularly limited as long as the skeleton is a known structure in the electrophotographic photoreceptor, and examples thereof include a structure conjugated with a nitrogen atom, which is a skeleton derived from a nitrogen-containing positive hole-transporting compound such as a triarylamine-based compound, a benzidine-based compound, or a hydrazone-based compound. Among these, for example, a triarylamine skeleton is preferable.

The reactive group-containing charge transport material having the reactive group and the charge-transporting skeleton, the non-reactive charge transport material, and the reactive group-containing non-charge transport material may be selected from known materials.

The protective layer may also contain other known additives.

The formation of the protective layer is not particularly limited, and a known forming method is used. For example, a coating film of a coating solution for forming a protective layer in which the above-described components are added to a solvent is formed, and the coating film is dried and, as necessary, subjected to a curing treatment such as heating.

Examples of the solvent for preparing the coating solution for forming a protective layer include an aromatic solvent such as toluene or xylene; a ketone-based solvent such as methyl ethyl ketone, methyl isobutyl ketone, or cyclohexanone; an ester-based solvent such as ethyl acetate or butyl acetate; an ether-based solvent such as tetrahydrofuran or dioxane; a cellosolve-based solvent such as ethylene glycol monomethyl ether; and an alcohol-based solvent such as isopropyl alcohol or butanol. These solvents are used alone or in the form of a mixture of two or more kinds thereof.

**In** addition, the coating solution for forming a protective layer may be a solvent-less coating solution.

Examples of the method of coating the photosensitive layer (such as the charge transport layer) with the coating solution for forming a protective layer include typical coating methods such as a dip coating method, a push-up coating method, a wire bar coating method, a spray coating method, a blade coating method, an air knife coating method, and a curtain coating method.

The film thickness of the protective layer is set to be, for example, preferably in a range of 1 µm or greater and 20 µm or less and more preferably in a range of 2 µm or greater and 10 µm or less.

### [Single Layer Type Photosensitive Layer]

The single layer type photosensitive layer (charge generation/charge transport layer) is a layer containing a charge generation material, a charge transport material, a binder resin, and as necessary, other known additives. Further, these materials are the same as the materials described in the sections of the charge generation layer and the charge transport layer.

Further, the content of the charge generation material in the single layer type photosensitive layer may be, for example, 0.1% by mass or greater and 10% by mass or less and preferably 0.8% by mass or greater and 5% by mass or less with respect to the total solid content. Further, the content of the charge transport material in the single layer type photosensitive layer may be, for example, 5% by mass or greater and 50% by mass or less with respect to the total solid content.

The method of forming the single layer type photosensitive layer is the same as the method of forming the charge generation layer or the charge transport layer.

The film thickness of the single layer type photosensitive layer may be, for example, 5 µm or greater and 50 µm or less and preferably 10 µm or greater and 40 µm or less.

### [Image Forming Apparatus and Process Cartridge]

An image forming apparatus according to the present exemplary embodiment includes the electrophotographic photoreceptor, a charging device that charges a surface of the electrophotographic photoreceptor, an electrostatic latent image forming device that forms an electrostatic latent image on the charged surface of the electrophotographic photoreceptor, a developing device that develops the electrostatic latent image formed on the surface of the electrophotographic photoreceptor with a developer containing a toner to form a toner image, and a transfer device that transfers the toner image to a surface of a recording medium. Further, the electrophotographic photoreceptor according to the present exemplary embodiment is employed as the electrophotographic photoreceptor.

As the image forming apparatus according to the present exemplary embodiment, known image forming apparatuses such as an apparatus including a fixing device that fixes a toner image transferred to the surface of a recording medium; a direct transfer type apparatus that transfers a toner image formed on the surface of an electrophotographic photoreceptor directly to a recording medium; an intermediate transfer type apparatus that primarily transfers a toner image formed on the surface of an electrophotographic photoreceptor to the surface of an intermediate transfer member and secondarily transfers the toner image transferred to the surface of the intermediate transfer member to the surface of a recording medium; an apparatus including a cleaning device that cleans the surface of an electrophotographic photoreceptor after the transfer of a toner image and before the charging; an apparatus including a charge erasing device that erases the charges on the surface of an electrophotographic photoreceptor by applying the charge erasing light after the transfer of a toner image and before the charging; and an apparatus including an electrophotographic photoreceptor heating member for increasing the temperature of an electrophotographic photoreceptor and decreasing the relative temperature are employed.

In a case of the intermediate transfer type apparatus, the transfer device is, for example, configured to include an intermediate transfer member having a surface onto which the toner image is transferred, a primary transfer device primarily transferring the toner image formed on the surface of the electrophotographic photoreceptor to the surface of the intermediate transfer member, and a secondary transfer device secondarily transferring the toner image transferred to the surface of the intermediate transfer member to the surface of the recording medium.

The image forming apparatus according to the present exemplary embodiment may be any of a dry development type image forming apparatus or a wet development type (development type using a liquid developer) image forming apparatus.

Further, in the image forming apparatus according to the present exemplary embodiment, for example, the portion including the electrophotographic photoreceptor may have a cartridge structure (process cartridge) that is attachable to and detachable from the image forming apparatus. As the process cartridge, for example, a process cartridge including the electrophotographic photoreceptor according to the present exemplary embodiment is preferably used. Further, the process cartridge may include, for example, at least one selected from the group consisting of a charging device, an electrostatic latent image forming device, a developing device, and a transfer device in addition to the electrophotographic photoreceptor.

Hereinafter, an example of the image forming apparatus according to the present exemplary embodiment will be described, but the present exemplary embodiment is not limited thereto. Further, main parts shown in the figures will be described, but description of other parts will not be provided.

Fig. 2 is a schematic configuration view showing an example of the image forming apparatus according to the present exemplary embodiment.

As shown in Fig. 2, an image forming apparatus 100 according to the present exemplary embodiment includes a process cartridge 300 including an electrophotographic photoreceptor 7, an exposure device 9 (an example of an electrostatic latent image forming device), a transfer device 40 (primary transfer device), and an intermediate transfer member 50. Further, in the image forming apparatus 100, the exposure device 9 is disposed at a position that can be exposed to the electrophotographic photoreceptor 7 from an opening portion of the process cartridge 300, the transfer device 40 is disposed at a position that faces the electrophotographic photoreceptor 7 via the intermediate transfer member 50, and the intermediate transfer member 50 is disposed such that a part of the intermediate transfer member 50 is in contact with the electrophotographic photoreceptor 7. Although not shown, the image forming apparatus also includes a secondary transfer device that transfers the toner image transferred to the intermediate transfer member 50 to a recording medium (for example, paper). Further, the intermediate transfer member 50, the transfer device 40 (primary transfer device), and the secondary transfer device (not shown) correspond to an example of the transfer device.

The process cartridge 300 in Fig. 2 integrally supports the electrophotographic photoreceptor 7, a charging device 8 (an example of the charging device), a developing device 11 (an example of the developing device), and a cleaning device 13 (an example of the cleaning device) in a housing. The cleaning device 13 has a cleaning blade (an example of the cleaning member) 131, and the cleaning blade 131 is disposed to come into contact with the surface of the electrophotographic photoreceptor 7. Further, the cleaning member may be a conductive or insulating fibrous member instead of the aspect of the cleaning blade 131, and may be used alone or in combination with the cleaning blade 131.

Further, Fig. 2 shows an example of an image forming apparatus including a fibrous member 132 (roll shape) that supplies a lubricant 14 to the surface of the electrophotographic photoreceptor 7 and a fibrous member 133 (flat brush shape) that assists cleaning, but these are disposed as necessary.

Hereinafter, each configuration of the image forming apparatus according to the present exemplary embodiment will be described.

### - Charging Device -

As the charging device 8, for example, a contact-type charger formed of a conductive or semi-conductive charging roller, a charging brush, a charging film, a charging rubber blade, a charging tube, or the like is used. Further, a known charger such as a non-contact type roller charger, or a scorotron charger or a corotron charger using corona discharge is also used.

### - Exposure Device -

Examples of the exposure device 9 include an optical system device that exposes the surface of the electrophotographic photoreceptor 7 to light such as a semiconductor laser beam, LED light, and liquid crystal shutter light in a predetermined image pattern. The wavelength of the light source is within the spectral sensitivity region of the electrophotographic photoreceptor. As the wavelength of a semiconductor laser, near infrared, which has an oscillation wavelength in the vicinity of 780 nm, is mostly used. However, the wavelength is not limited thereto, and a laser having an oscillation wavelength of an approximately 600 nm level or a laser having an oscillation wavelength of 400 nm or greater and 450 nm or less as a blue laser may also be used. Further, a surface emission type laser light source capable of outputting a multi-beam is also effective for forming a color image.

### - Developing Device -

Examples of the developing device 11 include a typical developing device that performs development in contact or non-contact with the developer. The developing device 11 is not particularly limited as long as the developing device has the above-described functions, and is selected depending on the purpose thereof. Examples of the developing device include known developing machines having a function of attaching a one-component developer or a two-component developer to the electrophotographic photoreceptor 7 using a brush, a roller, or the like. Among these, for example, a developing device formed of a developing roller having a surface on which a developer is held is preferably used.

The developer used in the developing device 11 may be a one-component developer containing only a toner or a two-component developer containing a toner and a carrier. Further, the developer may be magnetic or non-magnetic. Known developers are employed as these developers.

### - Cleaning Device -

As the cleaning device 13, a cleaning blade type device including the cleaning blade 131 is used.

In addition to the cleaning blade type device, a fur brush cleaning type device or a simultaneous development cleaning type device may be employed.

### - Transfer Device -

Examples of the transfer device 40 include a known transfer charger such as a contact type transfer charger using a belt, a roller, a film, or a rubber blade, and a scorotron transfer charger or a corotron transfer charger using corona discharge.

### - Intermediate Transfer Member -

As the intermediate transfer member 50, a belt-like intermediate transfer member (intermediate transfer belt) containing semi-conductive polyimide, polyamide-imide, polycarbonate, polyarylate, polyester, rubber, or the like is used. Further, as the form of the intermediate transfer member, a drum-like intermediate transfer member may be used in addition to the belt-like intermediate transfer member.

Fig. 3 is a schematic configuration view showing another example of the image forming apparatus according to the present exemplary embodiment.

An image forming apparatus 120 shown in Fig. 3 is a tandem type multicolor image forming apparatus on which four process cartridges 300 are mounted. The image forming apparatus 120 is formed such that four process cartridges 300 are arranged in parallel on the intermediate transfer member 50, and one electrophotographic photoreceptor is used for each color. Further, the image forming apparatus 120 has the same configuration as the image forming apparatus 100 except that the image forming apparatus 120 is of a tandem type.

### Examples

Hereinafter, the electrophotographic photoreceptor of the present disclosure will be described in more detail with reference to examples. The materials, the used amounts, the ratios, the treatment procedures, and the like described in the following examples may be appropriately changed without departing from the spirit of the present disclosure. Therefore, the scope of the electrophotographic photoreceptor of the present disclosure should not be limitatively interpreted by the specific examples described below.

### - Preparation of Undercoat Layer -

### (Preparation of Undercoat Layer 1)

32 parts by mass of an electron transport material (P-1) is mixed into a solution obtained by dissolving 15 parts by mass of a curable urethane resin (thermosetting resin, blocked isocyanate CORONATE BI-301, manufactured by Tosoh Corporation, solid content of 75%) and 6.3 parts by mass of a butyral resin (S-LEC BL-S, manufactured by Sekisui Chemical Co., Ltd.) in 170 parts by mass of methyl ethyl ketone, and the solution is subjected to a dispersion treatment for 300 minutes with a sand mill using glass beads having a diameter of 1 mmφ, thereby obtaining a dispersion liquid.

The glass beads are separated by filtration, and 0.005 parts by mass of bismuth carboxylate (K-KAT XK-640, manufactured by King Industries, Inc.) is added to the obtained dispersion liquid as a catalyst, thereby obtaining a coating solution for forming an undercoat layer. An aluminum base material is dipped in and coated with the coating solution using a dip coating method, and the solution is dried and cured at 160°C for 60 minutes, thereby obtaining an undercoat layer 1 containing a curable urethane resin and an electron transport material represented by General Formula (P) and having a thickness of 10 µm.

### (Preparation of Undercoat Layer 2)

30 parts by mass of an electron transport material (P-1) is mixed into a solution obtained by dissolving 15 parts by mass of a resol type phenol resin (thermosetting resin, PL-2215, manufactured by Gunei Chemical Industry Co., Ltd.) and 5.0 parts by mass of a butyral resin (S-LEC BL-1, manufactured by Sekisui Chemical Co., Ltd.) in 120 parts by mass of methyl ethyl ketone and 60 parts by mass of isopropanol, and the solution is subjected to a dispersion treatment for 300 minutes with a sand mill using glass beads having a diameter of 1 mmφ, thereby obtaining a dispersion liquid.

The glass beads are separated by filtration, and 0.003 parts by mass of blocked sulfonic acid (Nacure 2500, manufactured by King Industries, Inc.) is added to the obtained dispersion liquid as a catalyst, thereby obtaining a coating solution for forming an undercoat layer. An aluminum base material is dipped in and coated with the coating solution using a dip coating method, and the solution is dried and cured at 150°C for 60 minutes, thereby obtaining an undercoat layer 2 containing a phenol resin and an electron transport material represented by General Formula (P) and having a thickness of 10 µm.

### (Preparation of Undercoat Layer 3)

30 parts by mass of an electron transport material (P-1) is mixed into a solution obtained by dissolving 25 parts by mass of a methylated benzoguanamine resin (thermosetting resin, BL-60, manufactured by Sanwa Chemical Industrial Co., Ltd., solid content of 60%) and 5 parts by mass of methylated melamine (MW-390, manufactured by Sanwa Chemical Industrial Co., Ltd.) in 120 parts by mass of methyl ethyl ketone and 60 parts by mass of isopropanol, and the solution is subjected to a dispersion treatment for 300 minutes with a sand mill using glass beads having a diameter of 1 mmφ, thereby obtaining a dispersion liquid. The glass beads are separated by filtration, and 0.003 parts by mass of blocked sulfonic acid (Nacure 5225, manufactured by King Industries, Inc.) is added to the obtained dispersion liquid as a catalyst, thereby obtaining a coating solution for forming an undercoat layer. An aluminum base material is dipped in and coated with the coating solution using a dip coating method, and the solution is dried and cured at 150°C for 60 minutes, thereby obtaining an undercoat layer 3 containing a guanamine resin and an electron transport material represented by General Formula (P) and having a thickness of 10 µm.

### (Preparation of Undercoat Layer 4)

10 parts by mass of the electron transport material (P-1) having a primary particle diameter of 1 µm, 10 parts by mass of sodium chloride, and 150 parts by mass of 0.3 mm zirconia beads are added to a zirconia container, and the mixture is subjected to a pulverization treatment with a planetary mill (manufactured by Fritsch Japan Co., Ltd.) at 500 rpm for 1 hour. The zirconia beads are separated by filtration with a 50 µm mesh filter made of polypropylene and washed with methanol. The obtained crystals are repeatedly washed with distilled water and dried by a freeze dryer for 48 hours, thereby obtaining 7.5 parts by mass of an electron transport material (P-1). The treatment is repeated 4 times to obtain 30 parts by mass of a pulverized electron transport material (P-1) in total. The average primary particle diameter of 10 crystals randomly selected from a SEM image is 0.08 µm.

30 parts by mass of the obtained electron transport material (P-1), 15 parts by mass of a diallyl phthalate prepolymer (DAISO DAP (registered trademark) A, manufactured by Osaka Gas Co., Ltd.), 5.0 parts by mass of trimethylolpropane trimethacrylate, and 170 ml of methyl ethyl ketone are mixed and subjected to a dispersion treatment with a paint shaker using glass beads having a diameter of 1 mmφ for 180 minutes, thereby obtaining a dispersion liquid. 1.0 part by mass of PERBUTYL (registered trademark) Z (manufactured by NOF Corporation) serving as a polymerization initiator is added to the obtained dispersion liquid, thereby obtaining a coating solution for forming an undercoat layer. An aluminum base material is dipped in and coated with the coating solution using a dip coating method, and the solution is dried and cured at 160°C for 60 minutes in a nitrogen atmosphere, thereby obtaining an undercoat layer 4 containing a diallyl phthalate resin (thermosetting resin) and an electron transport material represented by General Formula (P) and having a thickness of 10 µm.

### (Preparation of Undercoat Layer 5)

30 g of the electron transport material (P-1) pulverized in the same manner as that for the undercoat layer 4 is added to a solution obtained by dissolving 20 g of nylon polyamide (thermoplastic resin, Amilan^{™} CM8000, manufactured by Toray Industries, Inc.) which is a copolymer of nylon and polyamide in 200 ml of methanol and subjected to a dispersion treatment with a paint shaker using glass beads having a diameter of 1 mmφ for 180 minutes, thereby obtaining a dispersion liquid. An aluminum base material is dipped in and coated with the coating solution using a dip coating method, and the solution is dried at 150°C for 45 minutes in a nitrogen atmosphere, thereby obtaining an undercoat layer 5 containing nylon polyamide and an electron transport material represented by General Formula (P) and having a thickness of 10 µm.

### (Preparation of Undercoat Layer 6)

An undercoat layer 6 is obtained in the same manner as in the preparation for the undercoat layer 1 except that the electron transport material (P-1) is changed to an electron transport material (P-3) in the undercoat layer 1.

### (Preparation of Undercoat Layer 7)

An undercoat layer 7 is obtained in the same manner as in the preparation for the undercoat layer 1 except that the electron transport material (P-1) is changed to an electron transport material (P-8) in the undercoat layer 1.

### (Preparation of Undercoat Layer 8)

An undercoat layer 8 is obtained in the same manner as in the preparation for the undercoat layer 1 except that the electron transport material (P-1) is changed to an electron transport material (P-1) pulverized in the same manner as that for the undercoat layer 4 in the undercoat layer 1.

### (Preparation of Undercoat Layer 9)

An undercoat layer 9 is obtained in the same manner as in the preparation for the undercoat layer 3 except that the methylated benzoguanamine resin is changed to a melamine resin (thermosetting resin, product name, MX-750, manufactured by Sanwa Chemical Industrial Co., Ltd.) in the undercoat layer 3.

### (Preparation of Undercoat Layers 10 to 14)

Each of the undercoat layers 10 to 14 is obtained in the same manner as in the preparation for the undercoat layer 1 except that the electron transport material (P-1) is changed to an electron transport material listed in Table 1 in the undercoat layer 1.

### (Preparation of Undercoat Layers 15 and 16)

Each of the undercoat layers 15 and 16 is obtained in the same manner as in the preparation for the undercoat layer 1 except that the thickness of the undercoat layer is changed to the thickness listed in Table 1 in the undercoat layer 1.

### (Preparation of Undercoat Layer 17)

An undercoat layer 17 is obtained in the same manner as in the preparation for the undercoat layer 1 except that the electron transport material (P-1) is changed to an electron transport material (P-1) having an average primary particle diameter of 0.01 µm which is obtained by setting the pulverization time to 4 hours in the preparation of the undercoat layer 4, in the undercoat layer 1.

### (Preparation of Undercoat Layer 18)

An undercoat layer 18 is obtained in the same manner as in the preparation for the undercoat layer 1 except that the electron transport material (P-1) is changed to an electron transport material (P-1) having a particle diameter of 1.2 µm which is obtained by recrystallization with sulfuric acid in the undercoat layer 1.

### (Preparation of Undercoat Layer 19)

32 parts by mass of the electron transport material (P-1) and 5 parts by mass of zinc oxide fine particles (manufactured by Tayca Corporation, average particle diameter of 75 nm, specific surface area of 14 m²/g) are mixed into a solution obtained by dissolving 15 parts by mass of a curable urethane resin (thermosetting resin, blocked isocyanate CORONATE BI-301, manufactured by Tosoh Corporation, solid content of 75%) and 6.3 parts by mass of a butyral resin (S-LEC BL-S, manufactured by Sekisui Chemical Co., Ltd.) in 170 parts by mass of methyl ethyl ketone, and the solution is subjected to a dispersion treatment for 300 minutes with a sand mill using glass beads having a diameter of 1 mmφ, thereby obtaining a dispersion liquid.

The glass beads are separated by filtration, and 0.005 parts by mass of bismuth carboxylate (K-KAT XK-640, manufactured by King Industries, Inc.) is added to the obtained dispersion liquid as a catalyst, thereby obtaining a coating solution for forming an undercoat layer. An aluminum base material is dipped in and coated with the coating solution using a dip coating method, and the solution is dried and cured at 160°C for 60 minutes, thereby obtaining an undercoat layer 19 containing a curable urethane resin and an electron transport material represented by General Formula (P) and having a thickness of 10 µm.

### (Preparation of Undercoat Layer 20)

An undercoat layer 20 is obtained in the same manner as in the preparation for the undercoat layer 1 except that the content of the electron transport material (P-1) is changed to the amount of the undercoat layer with respect to the total solid content listed in Table 1.

### (Preparation of Undercoat Layer 1 for Comparative Example)

An undercoat layer 1 for comparison is obtained in the same manner as in the preparation for the undercoat layer 1 except that the electron transport material (P-1) is changed to the imide compound (A) shown below in the undercoat layer 1.

### (Preparation of Undercoat Layer 2 for Comparative Example)

An undercoat layer 2 for comparison is obtained in the same manner as in the preparation for the undercoat layer 1 except that the electron transport material (P-1) is changed to the imide compound (B) shown below in the undercoat layer 1.

### (Preparation of Undercoat Layer 3 for Comparative Example)

An undercoat layer 3 for comparison is obtained in the same manner as in the preparation for the undercoat layer 1 except that the electron transport material (P-1) is changed to the imide compound (C) shown below in the undercoat layer 1.

### (Preparation of Undercoat Layer 4 for Comparative Example)

An undercoat layer 4 for comparison is obtained in the same manner as in the preparation for the undercoat layer 1 except that the electron transport material (P-1) is changed to the imide compound (C) shown below and the amount of the imide compound (C) is set as listed in Table 1 in the undercoat layer 1.

### <Examples 1 to 20 and Comparative Examples 1 to 4>

### (Formation of Charge Generation Layer)

A mixture of 15 parts by mass of hydroxygallium phthalocyanine having diffraction peaks at positions where Bragg angles (2θ ± 0.2°) in an X-ray diffraction spectrum using Cukα characteristic X-rays are at least 7.3°, 16.0°, 24.9°, and 28.0° as the charge generation material, 10 parts by mass of vinyl chloride-vinyl acetate copolymer resin (VMCH, manufactured by Nippon Unicar Company Limited) as a binder resin, and 200 parts by mass of n-butyl acetate is stirred and dispersed in a sand mill for 4 hours using glass beads having a diameter of 1 mmφ. 175 parts by mass of n-butyl acetate and 180 parts by mass of methyl ethyl ketone are added to the obtained dispersion liquid, and the mixture is stirred, thereby obtaining a coating solution for forming a charge generation layer. The outer peripheral surface of the undercoat layer of the kind listed in Table 1 is dipped in and coated with the coating solution for forming a charge generation layer, and the solution is dried at 150°C for 15 minutes, thereby forming a charge generation layer having a film thickness of 0.2 µm.

### (Formation of Charge Transport Layer)

38 parts by mass of the charge transport agent (HT-1) shown below, 10 parts by mass of the charge transport agent (HT-2) shown below, 52 parts by mass of the polycarbonate resin (A) (viscosity average molecular weight: 46,000) shown below, and 0.3 part by mass of a fluorine-containing graft polymer (GF-500, manufactured by Toagosei Co., Ltd.) as a dispersion assistant are added to and dissolved in 800 parts by mass of tetrahydrofuran, 8 parts by mass of ethylene tetrafluoride resin (LUBRON L5, manufactured by Daikin Industries, Ltd., average particle diameter of 300 nm) is added thereto and dispersed at 5,500 rpm for 2 hours using a homogenizer (ULTRA-TURRAX, manufactured by IKA Japan K.K.), thereby obtaining a coating solution for forming a charge transport layer. The charge generation layer is coated with the coating solution, and the solution is dried at 140°C for 40 minutes, thereby forming a charge transport layer having a film thickness of 30 µm. This charge transport layer is defined as an electrophotographic photoreceptor.

In the formulae, the numerical values denote the molar ratio (mol%).

### <Evaluation>

The electrophotographic photoreceptor of each example or each comparative example is mounted on a modified image forming apparatus DocuCentre C5570 (manufactured by FUJIFIILM Business Innovation Corporation), and the following evaluations are performed.

### - Evaluation of Charge Maintainability -

The electrophotographic photoreceptor is charged with an applied voltage of -710V in an environment of 10°C and 15% RH, and an initial charging potential V1 (before image output) on the outer peripheral surface of the electrophotographic photoreceptor before image output and a charging potential V2 on the outer peripheral surface of the electrophotographic photoreceptor after 30,000 sheets of 50% halftone images are printed are measured. Next, a difference between the potentials V1 - V2 is calculated and the evaluation is performed according to the following evaluation standards. Further, the ranks A and B are in acceptable levels.
A: Less than 20 V
B: 20 V or greater and less than 25 V
C: 25 V or greater and less than 30 V
D: 30V or greater and less than 35V in a problematic level
E: 35V or greater in a problematic level

### - Evaluation of Sticking of Foreign Matter -

The suppression of foreign matter from being stuck is evaluated using a phenomenon in which a current flows and spot-like image defects are generated in a case where carbon fibers penetrate through the photosensitive layer and the undercoat layer and reach the conductive substrate. Here, the charging potential is typically set to -700 V. Carbon fibers (average diameter of 7 µm, average length of 30 µm) are mixed with the developer in an amount set such that the density reaches 0.2% by mass, and 20,000 sheets of images having a density of 20% are continuously output on A4 paper. Next, 10 sheets of images having a density of 20% are output on A4 paper. The presence or absence of spot-like image defects in the image of the 10th sheet is visually observed, and the degree of image defects is classified into A to D described below. The results are listed in Table 1.
A: Spot-like image defects are not found.
B: The number of spot-like image defects is less than 5.
C: The number of spot-like image defects is 5 or greater and less than 10.
D: The number of spot-like image defects is 10 or greater.

**[Table 1]**

| | Undercoat layer | | | | | | | | Evaluation | |
|---|---|---|---|---|---|---|---|---|---|---|
| | Type of undercoat layer | Binder resin | Electron transport material | | | | Thickness | Proportion of metal oxide | Evaluation of charge maintainability | Evaluation of sticking of foreign matter |
| | | Type | Type | Content | Average primary particle diameter | Aspect ratio | | | | |
| | | - | - | mass% | µm | - | µm | mass% | | |
| Example 1 | Undercoat layer 1 | Urethane resin | P-1 | 65 | 0.15 | 3.1 | 10 | 0 | A | A |
| Example 2 | Undercoat layer 2 | Phenol resin | P-1 | 65 | 0.15 | 3.1 | 10 | 0 | B | A |
| Example 3 | Undercoat layer 3 | Benzoguanamine resin | P-1 | 60 | 0.15 | 3.1 | 10 | 0 | A | A |
| Example 4 | Undercoat layer 4 | Diallyl phthalate resin | P-1 | 59 | 0.08 | 1.5 | 10 | 0 | B | A |
| Example 5 | Undercoat layer 5 | Nylon polyamide | P-1 | 60 | 0.15 | 3.1 | 10 | 0 | C | A |
| Example 6 | Undercoat layer 6 | Urethane resin | P-3 | 65 | 0.15 | 3.1 | 10 | 0 | B | A |
| Example 7 | Undercoat layer 7 | Urethane resin | P-8 | 65 | 0.15 | 3.1 | 10 | 0 | B | A |
| Example 8 | Undercoat layer 8 | Urethane resin | P-1 | 65 | 0.02 | 1.3 | 10 | 0 | B | A |
| Example 9 | Undercoat layer 9 | Urethane resin | P-1 | 60 | 0.15 | 2.6 | 10 | 0 | A | A |
| Example 10 | Undercoat layer 10 | Urethane resin | P-9 | 65 | 0.4 | 2.2 | 10 | 0 | C | A |
| Example 11 | Undercoat layer 11 | Urethane resin | P-10 | 65 | 0.21 | 1.7 | 10 | 0 | C | A |
| Example 12 | Undercoat layer 12 | Urethane resin | P-16 | 65 | 0.18 | 4 | 10 | 0 | C | A |
| Example 13 | Undercoat layer 13 | Urethane resin | P-12 | 65 | 0.1 | 2.8 | 10 | 0 | C | A |
| Example 14 | Undercoat layer 14 | Urethane resin | P-15 | 65 | 0.5 | 1.8 | 10 | 0 | C | A |
| Example 15 | Undercoat layer 15 | Urethane resin | P-1 | 65 | 0.15 | 3.1 | 18 | 0 | B | A |
| Example 16 | Undercoat layer 16 | Urethane resin | P-1 | 65 | 0.15 | 3.1 | 4 | 0 | A | C |
| Example 17 | Undercoat layer 17 | Urethane resin | P-1 | 65 | 0.01 | 1.1 | 10 | 0 | B | A |
| Example 18 | Undercoat layer 18 | Urethane resin | P-1 | 59 | 1.2 | 4 | 10 | 0 | C | A |
| Example 19 | Undercoat layer 19 | Urethane resin | P-1 | 59 | 0.15 | 3.1 | 10 | 9.2 | C | A |
| Example 20 | Undercoat layer 20 | Urethane resin | P-1 | 72 | 0.15 | 3.1 | 10 | 0 | A | A |
| Comparative example 1 | Undercoat layer 1 for comparison | Urethane resin | (A) | 65 | 0.15 | 3.3 | 10 | 0 | D | D |
| Comparative example 2 | Undercoat layer 2 for comparison | Urethane resin | (B) | 65 | 0.17 | 2 | 10 | 0 | D | D |
| Comparative example 3 | Undercoat layer 3 for comparison | Urethane resin | (C) | 65 | 0.2 | 1.5 | 10 | 0 | D | D |
| Comparative example 4 | Undercoat layer 4 for comparison | Urethane resin | (C) | 52 | 0.2 | 1.5 | 10 | 0 | E | D |

Further, it is found that the electrophotographic photoreceptors of the examples have excellent charge maintainability as compared with the electrophotographic photoreceptors of the comparative examples as listed in Table 1.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the appended claims.

### Brief Description of the Reference Symbols

1: undercoat layer
2: charge generation layer
3: charge transport layer
4: conductive substrate
5: photosensitive layer
7A: photoreceptor
7: electrophotographic photoreceptor
8: charging device
9: exposure device
11: developing device
13: cleaning device
14: lubricant
40: transfer device
50: intermediate transfer member
100: image forming apparatus
120: image forming apparatus
131: cleaning blade
132: fibrous member (roll shape)
133: fibrous member (flat brush shape)
300: process cartridge

## Claims

1. An electrophotographic photoreceptor (7) comprising:
a conductive substrate (4);
an undercoat layer (1) provided on the conductive substrate and containing a binder resin and an electron transport material represented by General Formula (P); and
a photosensitive layer (5) provided on the undercoat layer (1),
in General Formula (P), R¹, R², R³, R⁴, R⁵, R⁶, R⁷, and R⁸ each independently represent a hydrogen atom, an alkyl group, an alkoxy group, an aralkyl group, an aryl group, an alkoxycarbonyl group, or a halogen atom.

2. The electrophotographic photoreceptor (7) according to claim 1,
wherein in General Formula (P), R¹, R², R³, R⁴, R⁵, R⁶, R⁷, and R⁸ each independently represent a hydrogen atom or a halogen atom.

3. The electrophotographic photoreceptor (7) according to claim 1 or 2,
wherein in General Formula (P), R¹, R², R³, R⁴, R⁵, R⁶, R⁷, and R⁸ represent a hydrogen atom.

4. The electrophotographic photoreceptor (7) according to any one of claims 1 to 3,
wherein the electron transport material has an average primary particle diameter of 1 µm or less, the average primary particle diameter being determined in accordance with the method described the description.

5. The electrophotographic photoreceptor (7) according to claim 4,
wherein the electron transport material has an average primary particle diameter of 0.03 µm or greater and 1 µm or less.

6. The electrophotographic photoreceptor (7) according to any one of claims 1 to 5,
wherein a content of the electron transport material is less than 70% by mass with respect to a total solid content of the undercoat layer (1).

7. The electrophotographic photoreceptor (7) according to any one of claims 1 to 6,
wherein the undercoat layer (1) has a thickness of 5 µm or greater and 15 µm or less.

8. The electrophotographic photoreceptor according to any one of claims 1 to 7,
wherein the binder resin is a thermosetting resin.

9. The electrophotographic photoreceptor (7) according to claim 8,
wherein the thermosetting resin includes at least one resin selected from the group consisting of a urethane resin, a melamine resin, and a benzoguanamine resin.

10. The electrophotographic photoreceptor (7) according to claim 1,
wherein a content of a metal oxide in the undercoat layer (1) is 5% by mass or less with respect to a total solid content of the undercoat layer (1).

11. A process cartridge (300) comprising:
the electrophotographic photoreceptor (7) according to any one of claims 1 to 10,
wherein the process cartridge (300) is attachable to and detachable from an image forming apparatus (100).

12. An image forming apparatus (100) comprising:
the electrophotographic photoreceptor (7) according to any one of claims 1 to 10;
a charging device (8) that charges a surface of the electrophotographic photoreceptor (7);
an electrostatic latent image forming device (9) that forms an electrostatic latent image on the charged surface of the electrophotographic photoreceptor (7);
a developing device (11) that develops the electrostatic latent image formed on the surface of the electrophotographic photoreceptor (7) with a developer containing a toner to form a toner image; and
a transfer device (40) that transfers the toner image to a surface of a recording medium.

## Patentansprüche

1. Elektrophotographischer Photorezeptor (7), umfassend:
ein leitfähiges Substrat (4);
eine Unterbeschichtungsschicht (1), die auf dem leitfähigen Substrat vorgesehen ist und ein Bindemittelharz und ein Elektronentransportmaterial, das durch allgemeine Formel (P) dargestellt ist, enthält; und
eine lichtempfindliche Schicht (5), die auf der Unterbeschichtungsschicht (1) vorgesehen ist,
wobei in allgemeiner Formel (P) R¹, R², R³, R⁴, R⁵, R⁶, R⁷ und R⁸ jeweils unabhängig voneinander ein Wasserstoffatom, eine Alkylgruppe, eine Alkoxygruppe, eine Aralkylgruppe, eine Arylgruppe, eine Alkoxycarbonylgruppe oder ein Halogenatom darstellen.

2. Elektrophotographischer Photorezeptor (7) nach Anspruch 1,
wobei in allgemeiner Formel (P) R¹, R², R³, R⁴, R⁵, R⁶, R⁷ und R⁸ jeweils unabhängig voneinander ein Wasserstoffatom oder ein Halogenatom darstellen.

3. Elektrophotographischer Photorezeptor (7) nach Anspruch 1 oder 2,
wobei in allgemeiner Formel (P) R¹, R², R³, R⁴, R⁵, R⁶, R⁷ und R⁸ ein Wasserstoffatom darstellen.

4. Elektrophotographischer Photorezeptor (7) nach einem der Ansprüche 1 bis 3,
wobei das Elektronentransportmaterial einen durchschnittlichen Primärpartikeldurchmesser von 1 µm oder weniger aufweist, wobei der durchschnittliche Primärpartikeldurchmesser in Übereinstimmung mit dem in der Beschreibung beschriebenen Verfahren bestimmt wird.

5. Elektrophotographischer Photorezeptor (7) nach Anspruch 4,
wobei das Elektronentransportmaterial einen durchschnittlichen Primärpartikeldurchmesser von 0,03 µm oder größer und 1 µm oder kleiner aufweist.

6. Elektrophotographischer Photorezeptor (7) nach einem der Ansprüche 1 bis 5,
wobei ein Gehalt des Elektronentransportmaterials weniger als 70 Massen-% in Bezug auf einen Gesamtfeststoffgehalt der Unterbeschichtungsschicht (1) beträgt.

7. Elektrophotographischer Photorezeptor (7) nach einem der Ansprüche 1 bis 6,
wobei die Unterbeschichtungsschicht (1) eine Dicke von 5 µm oder größer und 15 µm oder kleiner aufweist.

8. Elektrophotographischer Photorezeptor nach einem der Ansprüche 1 bis 7,
wobei das Bindemittelharz ein duroplastisches Harz ist.

9. Elektrophotographischer Photorezeptor (7) nach Anspruch 8,
wobei das duroplastische Harz mindestens ein Harz, das aus der Gruppe, die aus einem Urethanharz, einem Melaminharz und einem Benzoguanaminharz besteht, ausgewählt ist, enthält.

10. Elektrophotographischer Photorezeptor (7) nach Anspruch 1,
wobei ein Gehalt eines Metalloxids in der Unterbeschichtungsschicht (1) 5 Massen-% oder weniger in Bezug auf einen Gesamtfeststoffgehalt der Unterbeschichtungsschicht (1) beträgt.

11. Prozesskartusche (300), umfassend:
den elektrophotographischen Photorezeptor (7) nach einem der Ansprüche 1 bis 10, wobei die Prozesskartusche (300) an einer Bilderzeugungsvorrichtung (100) anbringbar und von dieser lösbar ist.

12. Bilderzeugungsvorrichtung (100), umfassend:
den elektrophotographischen Photorezeptor (7) nach einem der Ansprüche 1 bis 10;
eine Ladevorrichtung (8), die eine Oberfläche des elektrophotographischen Photorezeptors (7) lädt;
eine Erzeugungsvorrichtung (9) für elektrostatisches latentes Bild, die ein elektrostatisches latentes Bild auf der geladenen Oberfläche des elektrophotographischen Photorezeptors (7) erzeugt;
eine Entwicklungsvorrichtung (11), die das elektrostatische latente Bild, das auf der Oberfläche des elektrophotographischen Photorezeptors (7) erzeugt wird, mit einem Entwickler, der einen Toner enthält, entwickelt, um ein Tonerbild zu erzeugen; und
eine Übertragungsvorrichtung (40), die das Tonerbild auf eine Oberfläche eines Aufzeichnungsmediums überträgt.

## Revendications

1. Photorécepteur électrophotographique (7) comprenant :
un substrat conducteur (4) ;
une couche de sous-couche (1) prévue sur le substrat conducteur et contenant une résine liant et un matériau de transport d'électrons représenté par Formule générale (P) ; et
une couche photosensible (5) prévue sur la couche de sous-couche (1),
dans Formule générale (P), R¹, R², R³, R⁴, R⁵, R⁶, R⁷ et R⁸ représentent chacun indépendamment un atome d'hydrogène, un groupe alkyle, un groupe alkoxy, un groupe aralkyle, un groupe aryle, un groupe alkoxycarbonyle ou un atome d'halogène.

2. Photorécepteur électrophotographique (7) selon la revendication 1,
dans lequel dans Formule générale (P), R¹, R², R³, R⁴, R⁵, R⁶, R⁷ et R⁸ représentent chacun indépendamment un atome d'hydrogène ou un atome d'halogène.

3. Photorécepteur électrophotographique (7) selon la revendication 1 ou la revendication 2,
dans lequel dans Formule générale (P), R¹, R², R³, R⁴, R⁵, R⁶, R⁷ et R⁸ représentent un atome d'hydrogène.

4. Photorécepteur électrophotographique (7) selon l'une quelconque des revendications 1 à 3,
dans lequel le matériau de transport d'électrons a un diamètre moyen de particules primaires de 1 µm ou inférieur, le diamètre moyen de particules primaires étant déterminé conformément à la méthode décrite dans la description.

5. Photorécepteur électrophotographique (7) selon la revendication 4,
dans lequel le matériau de transport d'électrons a un diamètre moyen de particules primaires de 0,03 µm ou supérieur et de 1 µm ou inférieur.

6. Photorécepteur électrophotographique (7) selon l'une quelconque des revendications 1 à 5,
dans lequel une teneur en matériau de transport d'électrons est inférieure à 70 % en masse par rapport à une teneur totale en solides de la couche de sous-couche (1).

7. Photorécepteur électrophotographique (7) selon l'une quelconque des revendications 1 à 6,
dans lequel la couche de sous-couche (1) a une épaisseur de 5 µm ou supérieure et de 15 µm ou inférieure.

8. Photorécepteur électrophotographique selon l'une quelconque des revendications 1 à 7,
dans lequel la résine liant est une résine thermodurcissable.

9. Photorécepteur électrophotographique (7) selon la revendication 8,
dans lequel la résine thermodurcissable inclut au moins une résine choisie dans le groupe constitué d'une résine uréthane, d'une résine mélamine et d'une résine benzoguanamine.

10. Photorécepteur électrophotographique (7) selon la revendication 1,
dans lequel une teneur en oxyde métallique dans la couche de sous-couche (1) est de 5 % en masse ou inférieure par rapport à une teneur totale en solides de la couche de sous-couche (1).

11. Cartouche de traitement (300) comprenant :
le photorécepteur électrophotographique (7) selon l'une quelconque des revendications 1 à 10, dans laquelle la cartouche de traitement (300) peut être fixée à et détachée d'un appareil de formation d'images (100).

12. Appareil de formation d'images (100) comprenant :
le photorécepteur électrophotographique (7) selon l'une quelconque des revendications 1 à 10 ;
un dispositif de charge (8) qui charge une surface du photorécepteur électrophotographique (7) ;
un dispositif de formation d'image latente électrostatique (9) qui forme une image latente électrostatique sur la surface chargée du photorécepteur électrophotographique (7) ;
un dispositif de développement (11) qui développe l'image latente électrostatique formée sur la surface du photorécepteur électrophotographique (7) avec un révélateur contenant un toner pour former une image de toner ; et
un dispositif de transfert (40) qui transfère l'image de toner sur une surface d'un support d'enregistrement.
